



US007662757B2

(12) **United States Patent**  
**Poirier et al.**

(10) **Patent No.:** **US 7,662,757 B2**  
(45) **Date of Patent:** **Feb. 16, 2010**

(54) **STABLE DEFOAMANT COMPOSITION  
CONTAINING GTL FLUID AND/OR  
HYDRODEWAXATE AND/OR  
HYDROISOMERIZED/CATALYTIC (AND/OR  
SOLVENT) DEWAXED FLUID AS DILUENT**

(75) Inventors: **Marc Andre Poirier**, Sarnia (CA);  
**Susan Marie Mattingly**, Carneys Point,  
NJ (US)

(73) Assignee: **ExxonMobil Research and  
Engineering Company**, Annandale, NJ  
(US)

(\*) Notice: Subject to any disclaimer, the term of this  
patent is extended or adjusted under 35  
U.S.C. 154(b) by 87 days.

(21) Appl. No.: **11/818,579**

(22) Filed: **Jun. 15, 2007**

(65) **Prior Publication Data**

US 2007/0298985 A1 Dec. 27, 2007

**Related U.S. Application Data**

(60) Provisional application No. 60/816,708, filed on Jun.  
27, 2006.

(51) **Int. Cl.**  
**B01D 19/04** (2006.01)

(52) **U.S. Cl.** ..... **508/207; 508/208; 508/215;**  
508/533; 516/123; 516/124

(58) **Field of Classification Search** ..... 208/18-19;  
508/107, 135, 207-208, 215, 533; 516/123-124  
See application file for complete search history.

(56) **References Cited**

**U.S. PATENT DOCUMENTS**

|                 |   |         |                      |         |
|-----------------|---|---------|----------------------|---------|
| 4,411,806 A     | * | 10/1983 | Tertiaux et al. .... | 508/208 |
| 4,584,115 A     |   | 4/1986  | Davis                |         |
| 5,766,513 A     | * | 6/1998  | Pillon et al. ....   | 516/123 |
| 6,090,758 A     |   | 7/2000  | Pillon et al.        |         |
| 6,090,989 A     | * | 7/2000  | Trewella et al. .... | 585/13  |
| 6,297,413 B1    | * | 10/2001 | Colson et al. ....   | 585/3   |
| 2005/0086854 A1 |   | 4/2005  | Millington et al.    |         |
| 2005/0109675 A1 |   | 5/2005  | Kremer               |         |
| 2005/0277794 A1 |   | 12/2005 | Cracknell et al.     |         |
| 2006/0025324 A1 |   | 2/2006  | Beetge et al.        |         |

**FOREIGN PATENT DOCUMENTS**

|    |                |         |
|----|----------------|---------|
| GB | 2 234 978 A    | 2/1991  |
| WO | WO 98/30306    | 1/1998  |
| WO | WO 00/14187    | 3/2000  |
| WO | WO 01/60955 A1 | *       |
| WO | WO 2005/021688 | 3/2005  |
| WO | WO 2006/135731 | 12/2006 |

\* cited by examiner

*Primary Examiner*—Robert J Hill, Jr.  
*Assistant Examiner*—Brian McCaig

(57) **ABSTRACT**

Defoamant solution exhibiting improved foam control performance over an extended time under ASTMD 892 or test method comprising base defoamant diluted in GTL fluid and/or hydrodewaxed waxy feed fluid and/or hydroisomerized/catalytic (and/or solvent) dewaxed waxy feed, the defoamant solution remaining clear with no separation over extended periods of time of storage prior to use.

**16 Claims, No Drawings**

## 1

**STABLE DEFOAMANT COMPOSITION  
CONTAINING GTL FLUID AND/OR  
HYDRODEWAXATE AND/OR  
HYDROISOMERIZED/CATALYTIC (AND/OR  
SOLVENT) DEWAXED FLUID AS DILUENT**

This application claims the benefit of U.S. Provisional Application 60/816,708 filed Jun. 27, 2006.

**FIELD OF THE INVENTION**

The present invention is directed to defoamants and especially solutions of defoamants, said defoamant solution comprising mixtures of the base defoamant diluted in a carrier fluid.

**BACKGROUND OF THE INVENTION**

The formation of foam in lubricating oils during use is undesirable because the presence of foam dramatically reduces the effectiveness of the lubricating oil, interfering with the ability of the lubricating oil to wet the surface being lubricated and interfering with the ability of the lubricating oil to carry off wear products, decomposition products, sludge, soot, and dissipate heat in the equipment being lubricated.

Foam formation in lubricating oils is counteracted by the use of defoamant. Defoamants function in part by being insoluble in the lubricant. The very characteristic which makes a material useful as a defoamant also has the negative effect of limiting the amount of defoamant that can be added to the lubricant to form a stable mixture, i.e., a mixture in which the defoamant remains in solution with the lubricant and does not separate out of the lubricant oil and therefore become ineffective for its intended purpose.

Numerous defoamants are known in the industry and have been employed with varying degrees of success. Defoamants include silicone anti-foam agents (or defoamants) such as polydimethylsiloxane (PDMS) oils and polymers thereof, silicone glycols, fluorinated PDMS and polyacrylate esters. Defoamants typically have kinematic viscosities at 25° C. in the range of from about 352 mm<sup>2</sup>/s to about 120,000 mm<sup>2</sup>/s and even higher.

**DESCRIPTION OF THE RELATED ART**

U.S. Pat. No. 5,766,513 teaches antifoam agents for use in automatic transmission fluids (ATFs). The antifoam agents are identified as polyacrylate and fluorosilicone, the antifoam agents being employed at very low levels.

GB 2,234,978 teaches polyacrylates or acrylic polymers as antifoam agents. Polyacrylates do not degrade the air release time of the oils to the same extent as PDMS and have replaced them in some application.

U.S. Pat. No. 6,090,758 teaches methods for reducing foam of a lubricating oil at both 24° C. and 93.5° C., the lubricating oil comprising a wax isomerate base oil, the anti-foam agent being polydimethylsiloxane having a viscosity at 25° C. in the range of 60,000 to 100,000 mm<sup>2</sup>/s and which exhibits a spreading coefficient of at least about 2 mN/m at both 24° C. and 93.5° C., used in an amount in the range of about 1 to 10 ppm.

U.S. Published Patent Application US2005/0109675 teaches that cross-linked polydimethylsiloxane (crosslinked PDMS) resins are useful as defoamers and antifoamants for

## 2

hydrocarbon-containing liquids. The PDMS resins are crosslinked with either alkylpolysiloxates or siloxane.

**DESCRIPTION OF THE INVENTION**

It has unexpectedly been found that defoamant/antifoam agents can be dissolved in a fluid selected from the group consisting of Gas-to-Liquids (GTL) fluid, hydrodewaxed, or hydroisomerized/catalytic (and/or solvent) dewaxed waxy feed origin fluids and mixtures thereof, preferably GTL fluid, to produce antifoam agent/defoamant solutions which remain stable for extended periods of time as evidenced by their remaining clear and bright and resisting the formation of "fish eyes", "clear and bright" and "fish eyes" or both subjective visual tests familiar to those skilled in the art. The GTL fluid, hydrodewaxed, or hydroisomerized/catalytic (and/or solvent) dewaxed waxy feed origin fluids or mixture thereof, preferably GTL fluid, useful in the present invention is/are characterized by boiling in the range of about 300° F. to about 750° F. (149° C. to 399° C.), preferable about 320° F. to about 734° F. (160° C. to 390° C.), more preferably about 320° F. to 700° F. (160° C. to 371° C.) the ranges recited corresponding to the initial boiling point (IBP) and to the final boiling point (FBP) of the fluid.

The GTL fluid and/or hydrodewaxed and/or hydroisomerized/catalytic (and/or solvent) dewaxed waxy feed derived fluid, preferably GTL fluid, useful as diluent is also characterized by a Kinematic Viscosity (KV) at 40° C. (ASTM D 445) in the range of about 1.2 to 4.5 mm<sup>2</sup>/s, preferably about 1.7 to 3.0 mm<sup>2</sup>/s, most preferably about 1.9 to 2.5 mm<sup>2</sup>/s.

One or more antifoam agent(s)/defoamant(s) is (are) combined into the diluent in amounts in the range of from about 0.05 to 50 wt %, preferably about 0.1 to 30 wt %, still more preferably from about 0.1 to 5 wt % and most preferably from about 0.1 to 2.0 wt %.

The antifoam agent/defoamant-diluent solution can be used in finished lubricating oil composition in the range of about 0.001 to 0.5 wt %, preferably about 0.001 to 0.25 wt %, more preferably about 0.001 to 0.15 wt % based on the total weight of the finished lubricating oil composition.

The antifoam agent/defoamant-diluent solution is characterized as being clear and bright and resistant to "fish eye" formation for extended periods, evidence of stability which is critical for the antifoam agent/defoamant-diluent solution to be effective when added to lubricating oil formations in performing their intended function.

The antifoam agent/defoamant-diluent solution must be stable. The stability of the solution has a tremendous impact on the performance of the solution in the lubricating oil composition. Solutions which are hazy or exhibit the formation of "fish eyes" on standing are not stable and will not function effectively when added to lubricating oil formation composition. The formation of haze or of "fish eyes" indicates that the solution is not homogeneous and the antifoam agent/defoamant is not uniformly dissolved in the diluent. If the antifoam agent/defoamant is not uniformly dissolved or dispersed in the diluent (uniform dissolution or dispersion being evidenced by the solution being characterized as clear and bright and absent "fish eyes") the solution cannot be dispersed effectively when added to the lubricant in which the antifoam agents/defoamants per se are not soluble.

While the clear and bright criteria for the antifoam agent/defoamant-diluent solution cannot and is not seen by the industry as absolute evidence that a given solution will necessarily function well in a lubricating oil formation composition, the presence of haze and/or "fish eye", i.e., the failure of the solution to be clear and bright is taken as a very good

indication that the solution will fail as an antifoamant/defoamant solution when added to a lubricating oil formulation composition.

Antifoamants/defoamants are not added directly to lube oil formulations because in most instances the antifoam agent/defoamant is either not soluble in or only slightly soluble in the base oil of the lubricating oil formulation composition.

It is suspected that antifoam agents/defoamants typically function effectively when the size of the dispersed antifoam agent/defoamant particle in the lubricating oil formulation composition has a parameter of about 2 to 10 microns.

As previously indicated, for the antifoam agent/defoamant to function effectively it must be dissolved in the oil. This is achieved by dissolving the antifoam agent/defoamant in a diluent, producing a stable solution and adding the stable solution to the lubricating oil formulation composition.

The antifoam agent/defoamant-diluent solution of the present invention can be added to any lubricating oil formulation composition comprising any natural, synthetic or non-conventional base stock/base oil, usually but not necessarily, also in combination with at least one additional performance enhancing additive.

Base stock is a lubricating oil that is manufactured by a single manufacturer to a particular specification regardless of feed stock source, manufacturer location or manufacturing technique and is identified by a unique designation. Base oils are one or more base stocks used to produce a particular lubricating oil product such as a formulated engine oil, etc.

The base stock of the formulated lubricating oil compositions can be any American Petroleum Institute (API) Groups I, II, III, IV or V base stocks. A wide range of lubricating base stocks is known in the art. Lubricating base stocks/base oils that can be benefited by the present invention are natural oils, synthetic oils, and unconventional oils of lubricating viscosity, typically those oils having a kinematic viscosity (KV) at 100° C. as measured by ASTM D445) in the range of about 2 to 100 mm<sup>2</sup>/s, preferably about 2 to 50 mm<sup>2</sup>/s, more preferably about 4 to 25 mm<sup>2</sup>/s. Natural oils, synthetic oils, and unconventional oils and mixtures thereof can be used unrefined, refined, or re-refined (the latter is also known as reclaimed or reprocessed oil). Unrefined oils are those obtained directly from a natural, synthetic or unconventional source and used without further purification. These include for example shale oil obtained directly from retorting operations, petroleum oil obtained directly from primary distillation, and ester oil obtained directly from an esterification process. Refined oils are similar to the oils discussed for unrefined oils except refined oils are subjected to one or more purification or transformation steps to improve at least one lubricating oil property. One skilled in the art is familiar with many purification or transformation processes. These processes include, for example, solvent extraction, secondary distillation, acid extraction, base extraction, filtration, percolation, hydrogenation, hydrorefining, and hydrofinishing. Re-refined oils are obtained by processes analogous to refined oils, but employ an oil that has been previously used.

Groups I, II, III, IV and V are broad categories of base stocks developed and defined by the American Petroleum Institute (API Publication 1509; www.API.org). Group I base stocks have a viscosity index of between 80 to 120 contain greater than 0.03% sulfur and/or less than 90% saturates. Group II base stocks have a viscosity index of between about 80 to 120, contain less than or equal to 0.03% sulfur and greater than or equal to 90% saturates. Group III stocks have a viscosity index greater than or equal to about 120 contain less than or equal to 0.03% sulfur and greater than or equal to 90% saturates. Group IV includes polyalphaolefins (PAO).

Group V base stocks include base stocks not included in Groups I-IV. Table A summarizes properties of each of these five groups.

TABLE A

|    | Base Stock Properties                                   |                                                                                                                                        |                                        |                                      |
|----|---------------------------------------------------------|----------------------------------------------------------------------------------------------------------------------------------------|----------------------------------------|--------------------------------------|
|    | Saturates                                               | Sulfur                                                                                                                                 | Viscosity Index                        |                                      |
| 10 | Group I<br>Group II<br>Group III<br>Group IV<br>Group V | <90% and/or<br>≥90% and<br>≥90% and<br>Polyalphaolefins (PAO)<br>All other base oil stocks not included<br>in Groups I, II, III, or IV | >0.03% and<br>≤0.03% and<br>≤0.03% and | ≥80 and <120<br>≥80 and <120<br>≥120 |
| 15 |                                                         |                                                                                                                                        |                                        |                                      |

Natural oils include animal oils (lard oil, for example), vegetable oils (castor oil and olive oil, for example), and mineral oils. Animal and vegetable oils possessing favorable thermal-oxidative stability can be used. Of the natural oils, mineral oils are preferred. Mineral oil compositions vary widely as to their crude source, for example, as to whether they are paraffinic, naphthenic, or mixed paraffinic-naphthenic. Oils derived from coal or oil shale are also useful in the present invention. Natural oils vary also as to the method used for their production and purification, for example, their distillation range and whether they are straight run or cracked, hydrorefined, or solvent extracted.

Synthetic oils include hydrocarbon oils as well as non-hydrocarbon oils. Synthetic oils can be derived from processes such as chemical combination (for example, polymerization, oligomerization, condensation, alkylation, acylation, etc.), where materials consisting of smaller, simpler molecular species are built up (i.e., synthesized) into materials consisting of larger, more complex molecular species. Synthetic oils include hydrocarbon oils such as polymerized and interpolymerized olefins (polybutylenes, polypropylenes, propylene isobutylene copolymers, ethylene-olefin copolymers, and ethylene-alphaolefin copolymers, for example). Polyalphaolefin (PAO) oil base stock is a commonly used synthetic hydrocarbon oil. By way of example, PAOs derived from C<sub>8</sub>, C<sub>10</sub>, C<sub>12</sub>, C<sub>14</sub> olefins or mixtures thereof may be utilized. See U.S. Pat. Nos. 4,956,122; 4,827,064; and 4,827,073.

The number average molecular weights of the PAOs, which are known materials and generally available on a major commercial scale from suppliers such as ExxonMobil Chemical Company, Chevron-Phillips, BP-Amoco, and others, typically vary from about 250 to about 3000, or higher, and PAOs may be made in kinematic viscosities up to about 100 cSt (measured at 100° C.), or higher. In addition, higher viscosity PAOs are commercially available, and may be made in kinematic viscosities up to about 3000 cSt (measured at 100° C.), or higher. The PAOs are typically comprised of relatively low molecular weight hydrogenated polymers or oligomers of alphaolefins which include, but are not limited to, about C<sub>2</sub> to about C<sub>32</sub> alphaolefins with about C<sub>8</sub> to about C<sub>16</sub> alphaolefins, such as 1-octene, 1-decene, 1-dodecene and the like, being preferred. The preferred polyalphaolefins are poly-1-octene, poly-1-decene and poly-1-dodecene and mixtures thereof and mixed olefin-derived polyolefins. Depending on the viscosity grade and the starting oligomer, the PAOs may be predominantly trimers and tetramers of the starting olefins, with minor amounts of the higher oligomers, having a viscosity range of about 1.5 to 12 cSt at 100° C. However, the dimers of higher olefins in the range of about C<sub>14</sub> to C<sub>18</sub> may be used to provide low viscosity base stocks of acceptably low volatility.

PAO fluids may be conveniently made by the polymerization of an alphaolefin in the presence of a polymerization catalyst such as the Friedel-Craft catalyst including, for example, aluminum trichloride, boron trifluoride or complexes of boron trifluoride with water, alcohols such as ethanol, propanol or butanol, carboxylic acids or esters such as ethyl acetate or ethyl propionate. For example the methods disclosed by U.S. Pat. No. 4,149,178 or U.S. Pat. No. 3,382,291 may be conveniently used herein. Other descriptions of PAO synthesis are found in the following U.S. Pat. Nos. 3,742,082; 3,769,363; 3,876,720; 4,239,930; 4,367,352; 4,413,156; 4,434,408; 4,910,355; 4,956,122; and 5,068,487. The dimers of the C<sub>14</sub> to C<sub>18</sub> olefins are described in U.S. U.S. Pat. No. 4,218,330.

Other useful synthetic lubricating base stock oils such as silicon-based oil or esters of phosphorus containing acids may also be utilized. For examples of other synthetic lubricating base stocks are the seminal work "Synthetic Lubricants", C. R. Gunderson and A. W. Hart, Reinhold Publishing Corp., New York, N.Y. (1962).

In alkylated aromatic stocks, the alkyl substituents are typically alkyl groups of about 8 to 25 carbon atoms, usually from about 10 to 18 carbon atoms and up to about three such substituents may be present, as described for the alkyl benzenes in ACS Petroleum Chemistry Preprint 1053-1058, "Poly n-Alkylbenzene Compounds: A Class of Thermally Stable and Wide Liquid Range Fluids", K. C. Eapen et al, Philadelphia (1984). Tri-alkyl benzenes may be produced by the cyclodimerization of 1-alkynes of 8 to 12 carbon atoms as described in U.S. Pat. No. 5,055,626. Other alkylbenzenes are described in European Patent Application No. 168 534 and U.S. Pat. No. 4,658,072. Alkylbenzenes are used as lubricant base stocks, especially for low-temperature applications (arctic vehicle and machinery service, and refrigeration oils) and in papermaking oils. They are commercially available from producers of linear alkylbenzenes (LABs) such as Vista Chemical Co., Huntsman Chemical Co., Chevron Chemical Co., and Nippon Oil Co. Linear alkylbenzenes typically have good low pour points, low temperature viscosities and Viscosity Index (VI) values greater than about 100, together with good solvency for additives. Other alkylated aromatics which may be used when desirable are described, for example, in "Synthetic Lubricants and High Performance Functional Fluids", H. Dressler, Chapter 5, (R. L. Shubkin (Ed.)), Marcel Dekker, New York, N.Y. (1993).

Alkylene oxide polymers and interpolymers and their derivatives containing modified terminal hydroxyl groups obtained by, for example, esterification or etherification are useful synthetic lubricating oils. By way of example, these oils may be obtained by polymerization of ethylene oxide, propylene oxide, or other alkylene oxides. The alkyl and aryl ethers of these polyoxyalkylene polymers (methyl-polyisopropylene glycol ether having an average molecular weight of about 1000, diphenyl ether of polyethylene glycol having a molecular weight of about 500-1000, and the diethyl ether of polypropylene glycol having a molecular weight of about 1000 to 1500, for example) or mono- and polyarboxylic esters thereof (the acidic acid esters, mixed C<sub>3-8</sub> fatty acid esters, or the C<sub>13</sub>Oxo acid diester of tetraethylene glycol, for example) can be used as lubricant base stocks.

Esters comprise useful base stocks. Additive solvency and seal swell characteristics may be secured by the use of esters such as the esters of dibasic acids with monoalkanols and the polyol esters of monocarboxylic acids. Esters of the former type include, for example, the esters of dicarboxylic acids such as phthalic acid, succinic acid, alkyl succinic acid, alkyl succinic acid, maleic acid, azelaic acid, suberic acid,

sebacic acid, fumaric acid, adipic acid, linoleic acid dimer, malonic acid, alkyl malonic acid, alkenyl malonic acid, etc., with a variety of alcohols such as butyl alcohol, hexyl alcohol, dodecyl alcohol, 2-ethylhexyl alcohol, etc. Specific examples of these types of esters include dibutyl adipate, di(2-ethylhexyl) sebacate, di-n-hexyl fumarate, dioctyl sebacate, diisooctyl azelate, diisodecyl azelate, dioctyl phthalate, didecyl phthalate, dieicosyl sebacate, etc.

Particularly useful synthetic esters are those which are obtained by reacting one or more polyhydric alcohols, preferably the hindered polyols such as the neopentyl polyols e.g. neopentyl glycol, trimethylol ethane, 2-methyl-2-propyl-1,3-propanediol, trimethylol propane, pentaerythritol and dipentaerythritol with alkanoic acids containing at least about 4 carbon atoms, preferably C<sub>5</sub> to C<sub>30</sub> acids such as saturated straight chain fatty acids including caprylic acid, capric acid, lauric acid, myristic acid, palmitic acid, stearic acid, arachic acid, and behenic acid, or the corresponding branched chain fatty acids or unsaturated fatty acids such as oleic acid.

Suitable synthetic ester base stock components include the esters of trimethylol propane, trimethylol butane, trimethylol ethane, pentaerythritol and/or dipentaerythritol with one or more monocarboxylic acids containing from about 5 to about 10 carbon atoms.

Silicon-based oils are another class of useful synthetic lubricating oils. These oils include polyalkyl-, polyaryl-, polyalkoxy-, and polyaryloxy-siloxane oils and silicate oils. Examples of suitable silicon-based oils include tetraethyl silicate, tetraisopropyl silicate, tetra-(2-ethylhexyl) silicate, tetra-(4-methylhexyl) silicate, tetra-(p-tert-butylphenyl) silicate, hexyl-(4-methyl-2-pentoxy) disiloxane, poly(methyl) siloxanes, and poly-(methyl-2-methylphenyl) siloxanes.

Another class of synthetic lubricating oil is esters of phosphorous-containing acids. These include, for example, tricresyl phosphate, trioctyl phosphate, the diethyl ester of decaphosphonic acid.

Another class of oils includes polymeric tetrahydrofurans, their derivatives, and the like.

Other useful fluids of lubricating viscosity include non-conventional or unconventional base stocks that have been processed, preferably catalytically, or synthesized to provide high performance lubrication characteristics.

Non-conventional or unconventional base stocks/base oils which either form the base oil into which is added the above described antifoam additive/dispersant-diluent oil solution, or of which a particular portion boiling in the 300 to 750° F. range constitutes the diluent fluid itself, include one or more base stock(s)/base oils derived from one or more Gas-to-Liquids (GTL) materials, and/or as well as one or more hydrodewaxates or hydroisomerate/catalytic (and/or solvent) dewaxed base stock(s) and/or base oils derived from natural wax or waxy feeds, mineral and or non-mineral oil waxy feed stocks such as slack waxes (which are waxes recovered from waxy hydrocarbon oils by solvent dewaxing), natural waxes, and waxy stocks such as gas oils, waxy fuels hydrocracker bottoms, waxy raffinate, hydrocrackate, thermal crackates, or other mineral oil, or even non-petroleum oil derived waxy materials such as waxy materials received from coal liquefaction or shale oil, and mixtures of such base stocks and/or base oils.

As used herein, the following terms have the indicated meanings:

a) "wax"—hydrocarbonaceous material having a high pour point, typically existing as a solid at room temperature, i.e., at a temperature in the range from about 15° C. to 25° C., and consisting predominantly of paraffinic materials;

- b) "paraffinic" material: any saturated hydrocarbons, such as alkanes. Paraffinic materials may include linear alkanes, branched alkanes (iso-paraffins), cycloalkanes (cycloparaffins; mono-ring and/or multi-ring), and branched cycloalkanes;
- c) "hydroprocessing": a refining process in which a feedstock is heated with hydrogen at high temperature and under pressure, commonly in the presence of a catalyst, to remove and/or convert less desirable components and to produce an improved product;
- d) "hydrotreating": a catalytic hydrogenation process that converts sulfur- and/or nitrogen-containing hydrocarbons into hydrocarbon products with reduced sulfur and/or nitrogen content, and which generates hydrogen sulfide and/or ammonia (respectively) as byproducts; similarly, oxygen containing hydrocarbons can also be reduced to hydrocarbons and water;
- e) "catalytic dewaxing": a conventional catalytic process in which normal paraffins (wax) and/or waxy hydrocarbons, e.g., slightly branched iso-paraffins, are converted by cracking/fragmentation into lower molecular weight species to insure that the final oil product (base stock or base oil) has the desired product pour point;
- f) "solvent dewaxing": a process whereby wax is physically removed from oil by use of chilled solvent or an autorefrigeration solvent to solidify the wax which can then be removed from the oil;
- g) "hydroisomerization" (or isomerization): a catalytic process in which normal paraffins (wax) and/or slightly branched iso-paraffins are converted by rearrangement/ isomerization into branched or more branched iso-paraffins (the isomerate from such a process possibly requiring a subsequent additional wax removal step to ensure that the final oil product (base stock or base oil) has the desired product pour point);
- h) "hydrocracking": a catalytic process in which hydrogenation accompanies the cracking/fragmentation of hydrocarbons, e.g., converting heavier hydrocarbons into lighter hydrocarbons, or converting aromatics and/or cycloparaffins (naphthenes) into non-cyclic branched paraffins.
- i) "hydrodewaxing": (e.g., ISODEWAXING® of Chevron or MSDW™ of Exxon Mobil corporation) a very selective catalytic process which in a single step or by use of a single catalyst or catalyst mixture effects conversion of wax by isomerization/rearrangement of the n-paraffins and slightly branched isoparaffins into more heavily branched isoparaffins, the resulting product not requiring a separate conventional catalytic or solvent dewaxing step to meet the desired product pour point;
- j) the terms "hydroisomerate", "isomerate", "catalytic dewaxate", and "hydrodewaxate" refer to the products produced by the respective processes, unless otherwise specifically indicated;
- k) "base stock" is a single oil secured from a single feed stock source and subjected to a single processing scheme and meeting a particular specification;
- l) "base oil" comprises one or more base stock(s).

Thus the term "hydroisomerization/(catalytic) dewaxing" is used to refer to catalytic processes which have the combined effect of converting normal paraffins and/or waxy hydrocarbons by rearrangement/isomerization, into more branched iso-paraffins, followed by (1) catalytic dewaxing to reduce the amount of any residual n-paraffins or slightly branched iso-paraffins present in the isomerate by cracking/fragmentation or by (2) hydrodewaxing to effect further isomerization and very selective catalytic dewaxing of the isomerate, to reduce the product pour point. When the term

"(and/or solvent)", is included in the recitation, the process described involves hydroisomerization followed by solvent dewaxing (or a combination of solvent dewaxing and catalytic dewaxing) which effects the physical separation of wax from the hydroisomerate so as to reduce the product pour point.

GTL materials are materials that are derived via one or more synthesis, combination, transformation, rearrangement, and/or degradation/deconstructive processes from gaseous carbon-containing compounds, hydrogen-containing compounds, and/or elements as feedstocks such as hydrogen, carbon dioxide, carbon monoxide, water, methane, ethane, ethylene, acetylene, propane, propylene, propyne, butane, butylenes, and butynes. GTL base stocks and/or base oils are GTL materials of lubricating viscosity that are generally derived from hydrocarbons, for example waxy synthesized hydrocarbons, that are themselves derived from simpler gaseous carbon-containing compounds, hydrogen-containing compounds and/or elements as feedstocks. GTL base stock(s) and/or base oil(s) include oils boiling in the lube oil boiling range separated/fractionated from synthesized GTL materials such as for example, by distillation and subsequently subjected to a final wax processing step which is either or both of the well-known catalytic dewaxing process, or solvent dewaxing process, to produce lube oils of reduced/low pour point; synthesized wax isomerates, comprising, for example, hydrodewaxed, or hydroisomerized/cat (and/or solvent) dewaxed synthesized waxy hydrocarbons; hydrodewaxed, or hydroisomerized/cat (and/or solvent) dewaxed Fischer-Tropsch (F-T) material (i.e., hydrocarbons, waxy hydrocarbons, waxes and possible analogous oxygenates); preferably hydrodewaxed, or hydroisomerized/cat (and/or solvent) dewaxed F-T hydrocarbons, or hydrodewaxed or hydroisomerized/cat (or solvent) dewaxed, F-T waxes, hydrodewaxed, or hydroisomerized/cat (and/or solvent) dewaxed synthesized waxes, or mixtures thereof.

GTL base stock(s) and/or base oil(s) derived from GTL materials, especially, hydrodewaxed, or hydroisomerized/cat (and/or solvent) dewaxed F-T material derived base stock(s) and/or base oil(s), and other hydrodewaxed, or hydroisomerized/cat (and/or solvent) dewaxed wax derived base stock(s) and/or base oil(s) are characterized typically as having kinematic viscosities at 100° C. of from about 2 mm<sup>2</sup>/s to about 50 mm<sup>2</sup>/s, preferably from about 3 mm<sup>2</sup>/s to about 50 mm<sup>2</sup>/s, more preferably from about 3.5 mm<sup>2</sup>/s to about 30 mm<sup>2</sup>/s, as exemplified by a GTL base stock derived by the hydrodewaxing or hydroisomerization/catalytic (or solvent dewaxing) of F-T wax, which has a kinematic viscosity of about 4 mm<sup>2</sup>/s at 100° C. and a viscosity index of about 130 or greater. The GTL fluid and/or hydrodewaxed and/or hydroisomerized/catalytic (and/or solvent) dewaxed wax derived fluid, preferably GTL fluid, suitable for use as the diluent fluid in the present invention has/have kinematic viscosity(ies) at 40° C. in the range of about 1.2 to 4.5 mm<sup>2</sup>/s, preferably about 1.7 to 3.0 mm<sup>2</sup>/s more preferably about 1.9 to 2.5 mm<sup>2</sup>/s. Preferably the wax treatment process is hydrodewaxing carried out in a process using a single hydrodewaxing catalyst. Reference herein to Kinematic viscosity refers to a measurement made by ASTM method D445.

GTL base stock(s) and/or base oil(s) derived from GTL materials, especially hydrodewaxed, or hydroisomerized/cat (and/or solvent) dewaxed F-T material derived base stock(s) and/or base oil(s), and other hydrodewaxed, or hydroisomerized/cat (and/or solvent) dewaxed wax-derived base stock(s) and/or base oil(s), which can be used as base stock and/or base oil components of this invention are further characterized typically as having pour points of about -5° C. or lower,

preferably about -10° C. or lower, more preferably about -15° C. or lower, still more preferably about -20° C. or lower, and under some conditions may have advantageous pour points of about -25° C. or lower, with useful pour points of about -30° C. to about -40° C. or lower. If necessary, a separate dewaxing step may be practiced to achieve the desired pour point. References herein to pour point refer to measurement made by ASTM D97 and similar automated versions.

The GTL base stock(s) and/or base oil(s) derived from GTL materials, especially hydrodewaxed or hydroisomerized/cat (and/or solvent) dewaxed F-T material derived base stock(s) and/or base oil(s), and other such wax-derived base stock(s) and/or base oil(s) which can be used in this invention are also characterized typically as having viscosity indices of 80 or greater, preferably 100 or greater, and more preferably 120 or greater. Additionally, in certain particular instances, the viscosity index of these base stocks and/or base oil(s) may be preferably 130 or greater, more preferably 135 or greater, and even more preferably 140 or greater. For example, GTL base stock(s) and/or base oil(s) that derive from GTL materials preferably F-T materials especially F-T wax generally have a viscosity index of 130 or greater. References herein to viscosity index refer to ASTM method D2270.

In addition, the GTL base stock(s) and/or base oil(s) are typically highly paraffinic (>90% saturates), and may contain mixtures of monocycloparaffins and multicycloparaffins in combination with non-cyclic isoparaffins. The ratio of the naphthenic (i.e., cycloparaffin) content in such combinations varies with the catalyst and temperature used. Further, GTL base stock(s) and/or base oil(s) typically have very low sulfur and nitrogen content, generally containing less than about 10 ppm, and more typically less than about 5 ppm of each of these elements. The sulfur and nitrogen content of GTL base stock(s) and/or base oil(s) obtained by the hydroisomerization/isodewaxing of F-T material, especially F-T wax, is essentially nil.

In a preferred embodiment, the GTL base stock(s) and/or base oil(s) comprises paraffinic materials that consist predominantly of non-cyclic isoparaffins and only minor amounts of cycloparaffins. These GTL base stock(s) and/or base oil(s) typically comprise paraffinic materials that consist of greater than 60 wt % non-cyclic isoparaffins, preferably greater than 80 wt % non-cyclic isoparaffins, more preferably greater than 85 wt % non-cyclic isoparaffins, and most preferably greater than 90 wt % non-cyclic isoparaffins.

Useful compositions of GTL base stock(s) and/or base oil(s), hydrodewaxed or hydroisomerized/cat (and/or solvent) dewaxed F-T material derived base stock(s), and wax-derived hydrodewaxed, or hydroisomerized/cat (and/or solvent) dewaxed base stock(s), such as wax isomerates or hydrodewaxates, are recited in U.S. Pat. Nos. 6,080,301; 6,090,989, and 6,165,949 for example.

Base stock(s) and/or base oil(s) derived from waxy feeds, which are also suitable for use in this invention, are paraffinic fluids of lubricating viscosity derived from hydrodewaxed, or hydroisomerized/cat (and/or solvent) dewaxed waxy feedstocks of mineral oil, non-mineral oil, non-petroleum, or natural source origin, e.g., feedstocks such as one or more of gas oils, slack wax, waxy fuels hydrocracker bottoms, hydrocarbon raffinates, natural waxes, hydrocrackates, thermal crackates, foots oil, wax from coal liquefaction or from shale oil, or other suitable mineral oil, non-mineral oil, non-petroleum, or natural source derived waxy materials, linear or branched hydrocarbyl compounds with carbon number of

about 20 or greater, preferably about 30 or greater, and mixtures of such isomerate/isodewaxate base stock(s) and/or base oil(s).

Slack wax is the wax recovered from any waxy hydrocarbon oil including synthetic oil such as F-T waxy oil or petroleum oils by solvent or autorefrigerative dewaxing. Solvent dewaxing employs chilled solvent such as methyl ethyl ketone (MEK), methyl isobutyl ketone (MIBK), mixtures of MEK/MIBK, mixtures of MEK and toluene, while autorefrigerative dewaxing employs pressurized, liquefied low boiling hydrocarbons such as propane or butane.

Slack wax(es) secured from synthetic waxy oils such as F-T waxy oil will usually have zero or nil sulfur and/or nitrogen containing compound content. Slack wax(es) secured from petroleum oils, may contain sulfur and nitrogen containing compounds. Such heteroatom compounds must be removed by hydrotreating (and not hydrocracking), as for example by hydrodesulfurization (HDS) and hydrodenitrogenation (HDN) so as to avoid subsequent poisoning/deactivation of the hydroisomerization catalyst.

The term GTL base stock and/or base oil and/or hydrodewaxate base stock and/or base oil and/or wax isomerate base stock and/or base oil as used herein and in the claims is to be understood as embracing individual fractions of GTL base stock and/or base oil and/or of wax-derived hydrodewaxed or hydroisomerized/cat (and/or solvent) dewaxed base stock and/or base oil as recovered in the production process, mixtures of two or more GTL base stock and/or base oil fractions and/or wax-derived hydrodewaxed, or hydroisomerized/cat (and/or solvent) dewaxed base stocks and/or base oil fractions, as well as mixtures of one or two or more low viscosity GTL base stock and/or base oil fraction(s) and/or wax-derived hydrodewaxed, or hydroisomerized/cat (and/or solvent) dewaxed base stock and/or base oil fraction(s) with one, two or more higher viscosity GTL base stock and/or base oil fraction(s) and/or wax-derived hydrodewaxed, or hydroisomerized/cat (and/or solvent) dewaxed base stock and/or base oil fraction(s) to produce a dumbbell blend wherein the blend exhibits a kinematic viscosity within the aforesaid recited range.

In a preferred embodiment, the GTL material, from which the GTL base stock(s) and/or base oil(s) is/are derived is an F-T material (i.e., hydrocarbons, waxy hydrocarbons, wax). A slurry F-T synthesis process may be beneficially used for synthesizing the feed from CO and hydrogen and particularly one employing an F-T catalyst comprising a catalytic cobalt component to provide a high Schultz-Flory kinetic alpha for producing the more desirable higher molecular weight paraffins. This process is also well known to those skilled in the art.

In an F-T synthesis process, a synthesis gas comprising a mixture of H<sub>2</sub> and CO is catalytically converted into hydrocarbons and preferably liquid hydrocarbons. The mole ratio of the hydrogen to the carbon monoxide may broadly range from about 0.5 to 4, but is more typically within the range of 55 from about 0.7 to 2.75 and preferably from about 0.7 to 2.5. As is well known, F-T synthesis processes include processes in which the catalyst is in the form of a fixed bed, a fluidized bed or as a slurry of catalyst particles in a hydrocarbon slurry liquid. The stoichiometric mole ratio for a F-T synthesis reaction is 2.0, but there are many reasons for using other than a stoichiometric ratio as those skilled in the art know. In cobalt slurry hydrocarbon synthesis process the feed mole ratio of the H<sub>2</sub> to CO is typically about 2.1/1. The synthesis gas comprising a mixture of H<sub>2</sub> and CO is bubbled up into the bottom of the slurry and reacts in the presence of the particulate F-T synthesis catalyst in the slurry liquid at conditions effective to form hydrocarbons, a portion of which are liquid

## 11

at the reaction conditions and which comprise the hydrocarbon slurry liquid. The synthesized hydrocarbon liquid is separated from the catalyst particles as filtrate by means such as filtration, although other separation means such as centrifugation can be used. Some of the synthesized hydrocarbons pass out the top of the hydrocarbon synthesis reactor as vapor, along with unreacted synthesis gas and other gaseous reaction products. Some of these overhead hydrocarbon vapors are typically condensed to liquid and combined with the hydrocarbon liquid filtrate. Thus, the initial boiling point of the filtrate may vary depending on whether or not some of the condensed hydrocarbon vapors have been combined with it. Slurry hydrocarbon synthesis process conditions vary somewhat depending on the catalyst and desired products. Typical conditions effective to form hydrocarbons comprising mostly  $C_{5+}$  paraffins, (e.g.,  $C_{5+}$ - $C_{200}$ ) and preferably  $C_{10+}$  paraffins, in a slurry hydrocarbon synthesis process employing a catalyst comprising a supported cobalt component include, for example, temperatures, pressures and hourly gas space velocities in the range of from about 320-850° F., 80-600 psi and 100-40,000 V/hr/V, expressed as standard volumes of the gaseous CO and H<sub>2</sub> mixture (0° C., 1 atm) per hour per volume of catalyst, respectively. The term " $C_{5+}$ " is used herein to refer to hydrocarbons with a carbon number of greater than 4, but does not imply that material with carbon number 5 has to be present. Similarly other ranges quoted for carbon number do not imply that hydrocarbons having the limit values of the carbon number range have to be present, or that every carbon number in the quoted range is present. It is preferred that the hydrocarbon synthesis reaction be conducted under conditions in which limited or no water gas shift reaction occurs and more preferably with no water gas shift reaction occurring during the hydrocarbon synthesis. It is also preferred to conduct the reaction under conditions to achieve an alpha of at least 0.85, preferably at least 0.9 and more preferably at least 0.92, so as to synthesize more of the more desirable higher molecular weight hydrocarbons. This has been achieved in a slurry process using a catalyst containing a catalytic cobalt component. Those skilled in the art know that by alpha is meant the Schultz-Flory kinetic alpha. While suitable F-T reaction types of catalyst comprise, for example, one or more Group VIII catalytic metals such as Fe, Ni, Co, Ru and Re, it is preferred that the catalyst comprise a cobalt catalytic component. In one embodiment the catalyst comprises catalytically effective amounts of Co and one or more of Re, Ru, Fe, Ni, Th, Zr, Hf, U, Mg and La on a suitable inorganic support material, preferably one which comprises one or more refractory metal oxides. Preferred supports for Co containing catalysts comprise Titania, particularly. Useful catalysts and their preparation are known and illustrative, but nonlimiting examples may be found, for example, in U.S. Pat. Nos. 4,568,663; 4,663,305; 4,542,122; 4,621,072 and 5,545,674.

As set forth above, the waxy feed from which the base stock(s) and/or base oil(s) is/are derived is a wax or waxy feed from mineral oil, non-mineral oil, non-petroleum, or other natural source, especially slack wax, or GTL material, preferably F-T material, referred to as F-T wax. F-T wax preferably has an initial boiling point in the range of from 650-750° F. and preferably continuously boils up to an end point of at least 1050° F. A narrower cut waxy feed may also be used during the hydroisomerization. A portion of the n-paraffin waxy feed is converted to lower boiling isoparaffinic material. Hence, there must be sufficient heavy n-paraffin material to yield an isoparaffin containing isomerate boiling in the lube oil range. If catalytic dewaxing is also practiced after isomerization/isodewaxing, some of the isomerate/isodewaxate will

## 12

also be hydrocracked to lower boiling material during the conventional catalytic dewaxing. Hence, it is preferred that the end boiling point of the waxy feed be above 1050° F. (1050° F.+).

5 When a boiling range is quoted herein it defines the lower and/or upper distillation temperature used to separate the fraction. Unless specifically stated (for example, by specifying that the fraction boils continuously or constitutes the entire range) the specification of a boiling range does not 10 require that any material at the specified limit has to be present, rather it excludes material boiling outside that range.

The waxy feed preferably comprises the entire 650-750° F.+ fraction formed by the hydrocarbon synthesis process, having an initial cut point between 650° F. and 750° F. determined by the practitioner and an end point, preferably above 15 1050° F., determined by the catalyst and process variables employed by the practitioner for the synthesis. Such fractions are referred to herein as "650-750° F.+ fractions". By contrast, "650-750° F.- fractions" refers to a fraction with an 20 unspecified initial cut point and an end point somewhere between 650° F. and 750° F. Waxy feeds may be processed as the entire fraction or as subsets of the entire fraction prepared by distillation or other separation techniques. The waxy feed also typically comprises more than 90%, generally more than 25 95% and preferably more than 98 wt % paraffinic hydrocarbons, most of which are normal paraffins. It has negligible amounts of sulfur and nitrogen compounds (e.g., less than 1 30 wppm of each), with less than 2,000 wppm, preferably less than 1,000 wppm and more preferably less than 500 wppm of oxygen, in the form of oxygenates. Waxy feeds having these properties and useful in the process of the invention have been made using a slurry F-T process with a catalyst having a catalytic cobalt component, as previously indicated.

The process of making the lubricant oil base stocks from 35 waxy stocks, e.g., slack wax or F-T wax, may be characterized as an isomerization process. If slack waxes are used as the feed, they may need to be subjected to a preliminary hydrotreating step under conditions already well known to those skilled in the art to reduce (to levels that would effectively avoid catalyst poisoning or deactivation) or to remove 40 sulfur- and nitrogen-containing compounds which would otherwise deactivate the hydroisomerization or hydrodewaxing catalyst used in subsequent steps. If F-T waxes are used, such preliminary treatment is not required because, as indicated above, such waxes have only trace amounts (less than 45 about 10 ppm, or more typically less than about 5 ppm to nil) of sulfur or nitrogen compound content. However, some hydrodewaxing catalyst fed F-T waxes may benefit from prehydrodreatment for the removal of oxygenates while others may benefit from oxygenates treatment. The hydroisomerization or hydrodewaxing process may be conducted over a combination of catalysts, or over a single catalyst. Conversion temperatures range from about 150° C. to about 500° C. at pressures ranging from about 500 to 20,000 kPa. 50 This process may be operated in the presence of hydrogen, and hydrogen partial pressures range from about 600 to 6000 kPa. The ratio of hydrogen to the hydrocarbon feedstock (hydrogen circulation rate) typically range from about 10 to 3500 n.1.l.<sup>-1</sup> (56 to 19,660 SCF/bbl) and the space velocity of the feedstock typically ranges from about 0.1 to 20 LHSV, 55 preferably 0.1 to 10 LHSV.

Following any needed hydrodenitrogenation or hydrodesulfurization, the hydroprocessing used for the production of base stocks from such waxy feeds may use an amorphous 60 hydrocracking/hydroisomerization catalyst, such as a lube hydrocracking (LHDC) catalysts, for example catalysts containing Co, Mo, Ni, W, Mo, etc., on oxide supports, e.g.,

alumina, silica, silica/alumina, or a crystalline hydrocracking/hydroisomerization catalyst, preferably a zeolitic catalyst.

Other isomerization catalysts and processes for hydrocracking, hydrodewaxing, or hydroisomerizing GTL materials and/or waxy materials to base stock or base oil are described, for example, in U.S. Pat. Nos. 2,817,693; 4,900,407; 4,937,399; 4,975,177; 4,921,594; 5,200,382; 5,516,740; 5,182,248; 5,290,426; 5,580,442; 5,976,351; 5,935,417; 5,885,438; 5,965,475; 6,190,532; 6,375,830; 6,332,974; 6,103,099; 6,025,305; 6,080,301; 6,096,940; 6,620,312; 6,676,827; 6,383,366; 6,475,960; 5,059,299; 5,977,425; 5,935,416; 4,923,588; 5,158,671; and 4,897,178; EP 0324528 (B1), EP 0532116 (B1), EP 0532118 (B1), EP 0537815 (B1), EP 0583836 (B2), EP 0666894 (B2), EP 0668342 (B1), EP 0776959 (A3), WO 97/031693 (A1), WO 02/064710 (A2), WO 02/064711 (A1), WO 02/070627 (A2), WO 02/070629 (A1), WO 03/033320 (A1) as well as in British Patents 1,429,494; 1,350,257; 1,440,230; 1,390,359; WO 99/45085 and WO 99/20720. Particularly favorable processes are described in European Patent Applications 464546 and 464547. Processes using F-T wax feeds are described in U.S. Pat. Nos. 4,594,172; 4,943,672; 6,046,940; 6,475,960; 6,103,099; 6,332,974; and 6,375,830.

Hydrocarbon conversion catalysts useful in the conversion of the n-paraffin waxy feedstocks disclosed herein to form the isoparaffinic hydrocarbon base oil are zeolite catalysts, such as ZSM-5, ZSM-11, ZSM-23, ZSM-35, ZSM-12, ZSM-38, ZSM-48, offretite, ferrierite, zeolite beta, zeolite theta, and zeolite alpha, as disclosed in U.S. Pat. No. 4,906,350. These catalysts are used in combination with Group VIII metals, in particular palladium or platinum. The Group VIII metals may be incorporated into the zeolite catalysts by conventional techniques, such as ion exchange.

In one embodiment, conversion of the waxy feedstock may be conducted over a combination of Pt/zeolite beta and Pt/ZSM-23 catalysts in the presence of hydrogen. In another embodiment, the process of producing the lubricant oil base stocks comprises hydroisomerization and dewaxing over a single catalyst, such as Pt/ZSM-35. In yet another embodiment, the waxy feed can be fed over a catalyst comprising Group VIII metal loaded ZSM-48, preferably Group VIII noble metal loaded ZSM-48, more preferably Pt/ZSM-48 in either one stage or two stages. In any case, useful hydrocarbon base oil products may be obtained. Catalyst ZSM-48 is described in U.S. Pat. No. 5,075,269. The use of the Group VIII metal loaded ZSM-48 family of catalysts, e.g., platinum on ZSM-48, in the hydroisomerization of the waxy feedstock eliminates the need for any subsequent, separate dewaxing step.

A dewaxing step, when needed, may be accomplished using one or more of solvent dewaxing, catalytic dewaxing or hydrodewaxing processes and either the entire hydroisomerate or the 650-750° F.+ fraction may be dewaxed, depending on the intended use of the 650-750° F.- material present, if it has not been separated from the higher boiling material prior to the dewaxing. In solvent dewaxing, the hydroisomerate may be contacted with chilled solvents such as acetone, methyl ethyl ketone (MEK), methyl isobutyl ketone (MIBK), mixtures of MEK/MIBK, or mixtures of MEK/toluene and the like, and further chilled to precipitate out the higher pour point material as a waxy solid which is then separated from the solvent-containing lube oil fraction which is the raffinate. The raffinate is typically further chilled in scraped surface chillers to remove more wax solids. Autorefrigerative dewaxing using low molecular weight hydrocarbons, such as propane, can also be used in which the hydroisomerate is

mixed with, e.g., liquid propane, a least a portion of which is flashed off to chill down the hydroisomerate to precipitate out the wax. The wax is separated from the raffinate by filtration, membrane separation or centrifugation. The solvent is then stripped out of the raffinate, which is then fractionated to produce the preferred base stocks useful in the present invention. Also well known is catalytic dewaxing, in which the hydroisomerate is reacted with hydrogen in the presence of a suitable dewaxing catalyst at conditions effective to lower the pour point of the hydroisomerate. Catalytic dewaxing also converts a portion of the hydroisomerate to lower boiling materials, in the boiling range, for example, 650-750° F.-, which are separated from the heavier 650-750° F.+ base stock fraction and the base stock fraction fractionated into two or more base stocks. Separation of the lower boiling material may be accomplished either prior to or during fractionation of the 650-750° F.+ material into the desired base stocks.

Any dewaxing catalyst which will reduce the pour point of the hydroisomerate and preferably those which provide a large yield of lube oil base stock from the hydroisomerate may be used. These include shape selective molecular sieves which, when combined with at least one catalytic metal component, have been demonstrated as useful for dewaxing petroleum oil fractions and include, for example, ferrierite, mordenite, ZSM-5, ZSM-11, ZSM-23, ZSM-35, ZSM-22 also known as theta one or TON, and the silicoaluminophosphates known as SAPO's. A dewaxing catalyst which has been found to be unexpectedly particularly effective comprises a noble metal, preferably Pt, composited with H-mordenite. The dewaxing may be accomplished with the catalyst in a fixed, fluid or slurry bed. Typical dewaxing conditions include a temperature in the range of from about 400-600° F., a pressure of 500-900 psig, H<sub>2</sub> treat rate of 1500-3500 SCF/B for flow-through reactors and LHSV of 0.1-10, preferably 0.2-2.0. The dewaxing is typically conducted to convert no more than 40 wt % and preferably no more than 30 wt % of the hydroisomerate having an initial boiling point in the range of 650-750° F. to material boiling below its initial boiling point.

GTL base stock(s) and/or base oil(s), hydrodewaxed, or hydroisomerized/cat (or solvent) dewaxed wax-derived base stock(s) and/or base oil(s), have a beneficial kinematic viscosity advantage over conventional API Group II and Group III base stock(s) and/or base oil(s), and so may be very advantageously used with the instant invention. Such GTL base stock(s) and/or base oil(s) can have significantly higher kinematic viscosities, up to about 20-50 mm<sup>2</sup>/s at 100° C., whereas by comparison commercial Group II base oils can have kinematic viscosities up to about 15 mm<sup>2</sup>/s at 100° C., and commercial Group III base oils can have kinematic viscosities up to about 10 mm<sup>2</sup>/s at 100° C. The higher kinematic viscosity range of GTL base stock(s) and/or base oil(s), compared to the more limited kinematic viscosity range of Group II and Group III base stock(s) and/or base oil(s), in combination with the instant invention can provide additional beneficial advantages in formulating lubricant compositions.

In the present invention mixtures of hydrodewaxate, or hydroisomerate/cat (or solvent) dewaxate base stock(s) and/or base oil(s), mixtures of the GTL base stock(s) and/or base oil(s), or mixtures thereof, preferably mixtures of GTL base stock(s) and/or base oil(s), can constitute all or part of the base stock which form the base oil of any formulated lubricating oil composition.

One or more of these waxy feed derived base stock(s) and/or base oil(s) derived from GTL materials and/or other waxy feed materials can be used as such or in further combination with other base stock(s) and/or base oil(s) of mineral

## 15

oil origin, natural oils and/or with synthetic base oils. The GTL base stock and/or base oil and/or hydrodewaxed and/or hydroisomerized/catalytic (and/or solvent) dewaxed waxy feed derived base stock(s) and/or base oil(s), preferably GTL base stock(s) and/or base oil(s), more preferably GTL base stock(s) and/or base oil(s) obtained from F-T waxy feed, still more preferably GTL base stock(s) and/or base oil(s) obtained by the hydrodewaxing or hydroisomerization/catalytic (and/or solvent) dewaxing of F-T wax, can constitute from about 5 to 100 wt %, preferably between about 20 to 40 to up to 100 wt %, more preferably about 70 to 100 wt % of the total of the base oil, the amount employed being left to the practitioner in response to the requirements of the finished lubricant.

The preferred base stock(s) and/or base oil(s) derived from GTL materials and/or from waxy feeds are characterized as having predominantly paraffinic compositions and are further characterized as having high saturates levels, low-to-nil sulfur, low-to-nil nitrogen, low-to-nil aromatics, and are essentially water-white in color.

A preferred GTL liquid hydrocarbon composition is one comprising paraffinic hydrocarbon components in which the extent of branching, as measured by the percentage of methyl hydrogens (BI), and the proximity of branching, as measured by the percentage of recurring methylene carbons which are four or more carbons removed from an end group or branch ( $\text{CH}_2 \geq 4$ ), are such that: (a)  $\text{BI} - 0.5(\text{CH}_2 \geq 4) > 15$ ; and (b)  $\text{BI} + 0.85(\text{CH}_2 \geq 4) < 45$  as measured over said liquid hydrocarbon composition as a whole.

The preferred GTL base stock and/or base oil can be further characterized, if necessary, as having less than 0.1 wt % aromatic hydrocarbons, less than 20 wppm nitrogen containing compounds, less than 20 wppm sulfur containing compounds, a pour point of less than  $-18^\circ\text{C}$ ., preferably less than  $-30^\circ\text{C}$ ., a preferred  $\text{BI} \geq 25.4$  and  $(\text{CH}_2 \geq 4) \leq 22.5$ . They have a nominal boiling point of  $370^\circ\text{C}.$ ., on average they average fewer than 10 hexyl or longer branches per 100 carbon atoms and on average have more than 16 methyl branches per 100 carbon atoms. They also can be characterized by a combination of dynamic viscosity, as measured by CCS at  $-40^\circ\text{C}.$ ., and kinematic viscosity, as measured at  $100^\circ\text{C}$ . represented by the formula: DV (at  $-40^\circ\text{C}.$ )  $< 2900$  (KV at  $100^\circ\text{C}.$ )  $- 7000$ .

The preferred GTL base stock and/or base oil is also characterized as comprising a mixture of branched paraffins characterized in that the lubricant base oil contains at least 90% of a mixture of branched paraffins, wherein said branched paraffins are paraffins having a carbon chain length of about  $\text{C}_{20}$  to about  $\text{C}_{40}$ , a molecular weight of about 280 to about 562, a boiling range of about  $650^\circ\text{F}$ . to about  $1050^\circ\text{F}$ ., and wherein said branched paraffins contain up to four alkyl branches and wherein the free carbon index of said branched paraffins is at least about 3.

In the above the Branching Index (BI), Branching Proximity ( $\text{CH}_2 \geq 4$ ), and Free Carbon Index (FCI) are determined as follows:

## Branching Index

A 359.88 MHz 1H solution NMR spectrum is obtained on a Bruker 360 MHz AMX spectrometer using 10% solutions in  $\text{CDCl}_3$ . TMS is the internal chemical shift reference.  $\text{CDCl}_3$  solvent gives a peak located at 7.28. All spectra are obtained under quantitative conditions using 90 degree pulse (10.9  $\mu\text{s}$ ), a pulse delay time of 30 s, which is at least five times the longest hydrogen spin-lattice relaxation time ( $T_1$ ), and 120 scans to ensure good signal-to-noise ratios.

H atom types are defined according to the following regions:

## 16

9.2-6.2 ppm hydrogens on aromatic rings;  
6.2-4.0 ppm hydrogens on olefinic carbon atoms;  
4.0-2.1 ppm benzylic hydrogens at the  $\alpha$ -position to aromatic rings;

5 2.1-1.4 ppm paraffinic CH methine hydrogens;  
1.4-1.05 ppm paraffinic  $\text{CH}_2$  methylene hydrogens;  
1.05-0.5 ppm paraffinic  $\text{CH}_3$  methyl hydrogens.  
The branching index (BI) is calculated as the ratio in percent of non-benzylic methyl hydrogens in the range of 0.5 to 1.05 ppm, to the total non-benzylic aliphatic hydrogens in the range of 0.5 to 2.1 ppm.

Branching Proximity ( $\text{CH}_2 \geq 4$ )

A 90.5 MHz  $^3\text{CMR}$  single pulse and 135 Distortionless Enhancement by Polarization Transfer (DEPT) NMR spectra are obtained on a Bruker 360 MHz AMX spectrometer using 10% solutions in  $\text{CDCl}_3$ . TMS is the internal chemical shift reference.  $\text{CDCl}_3$  solvent gives a triplet located at 77.23 ppm in the  $^{13}\text{C}$  spectrum. All single pulse spectra are obtained under quantitative conditions using 45 degree pulses (6.3  $\mu\text{s}$ ), a pulse delay time of 60 s, which is at least five times the longest carbon spin-lattice relaxation time ( $T_1$ ), to ensure complete relaxation of the sample, 200 scans to ensure good signal-to-noise ratios, and WALTZ-16 proton decoupling.

20 25 The C atom types  $\text{CH}_3$ ,  $\text{CH}_2$ , and  $\text{CH}$  are identified from the 135 DEPT  $^{13}\text{C}$  NMR experiment. A major  $\text{CH}_2$  resonance in all  $^{13}\text{C}$  NMR spectra at  $\approx 29.8$  ppm is due to equivalent recurring methylene carbons which are four or more removed from an end group or branch ( $\text{CH}_2 \geq 4$ ). The types of branches are determined based primarily on the  $^{13}\text{C}$  chemical shifts for the methyl carbon at the end of the branch or the methylene carbon one removed from the methyl on the branch.

30 35 The Free Carbon Index (FCI). The FCI is expressed in units of carbons, and is a measure of the number of carbons in an isoparaffin that are located at least 5 carbons from a terminal carbon and 4 carbons way from a side chain. Counting the terminal methyl or branch carbon as "one" the carbons in the FCI are the fifth or greater carbons from either a straight chain terminal methyl or from a branch methane carbon. These carbons appear between 29.9 ppm and 29.6 ppm in the carbon-13 spectrum. They are measured as follows:

- 40 45 a) calculate the average carbon number of the molecules in the sample which is accomplished with sufficient accuracy for lubricating oil materials by simply dividing the molecular weight of the sample oil by 14 (the formula weight of  $\text{CH}_2$ );  
50 b) divide the total carbon-13 integral area (chart divisions or area counts) by the average carbon number from step a. to obtain the integral area per carbon in the sample;  
c) measure the area between 29.9 ppm and 29.6 ppm in the sample; and  
d) divide by the integral area per carbon from step b. to obtain FCI.

55 60 Branching measurements can be performed using any Fourier Transform NMR spectrometer. Preferably, the measurements are performed using a spectrometer having a magnet of 7.0 T or greater. In all cases, after verification by Mass Spectrometry, UV or an NMR survey that aromatic carbons were absent, the spectral width was limited to the saturated carbon region, about 0-80 ppm vs. TMS (tetramethylsilane). Solutions of 15-25 percent by weight in chloroform-d1 were excited by 45 degrees pulses followed by a 0.8 sec acquisition time. In order to minimize non-uniform intensity data, the proton decoupler was gated off during a 10 sec delay prior to the excitation pulse and on during acquisition. Total experiment times ranged from 11-80 minutes. The DEPT and APT

sequences were carried out according to literature descriptions with minor deviations described in the Varian or Bruker operating manuals.

DEPT is Distortionless Enhancement by Polarization Transfer. DEPT does not show quaternaries. The DEPT 45 sequence gives a signal for all carbons bonded to protons. DEPT 90 shows CH carbons only. DEPT 135 shows CH and CH<sub>3</sub> up and CH<sub>2</sub> 180 degrees out of phase (down). APT is Attached Proton Test. It allows all carbons to be seen, but if CH and CH<sub>3</sub> are up, then quaternaries and CH<sub>2</sub> are down. The sequences are useful in that every branch methyl should have a corresponding CH and the methyls are clearly identified by chemical shift and phase. The branching properties of each sample are determined by C-13 NMR using the assumption in the calculations that the entire sample is isoparaffinic. Corrections are not made for n-paraffins or cycloparaffins, which may be present in the oil samples in varying amounts. The cycloparaffins content is measured using Field Ionization Mass Spectroscopy (FIMS).

GTL base stock(s) and/or base oil(s), and hydrodewaxed, or hydroisomerized/cat (or solvent) dewaxed wax base stock(s) and/or base oil(s), for example, hydrodewaxed or hydroisomerized/catalytic (and/or solvent) dewaxed waxy synthesized hydrocarbon, e.g., Fischer-Tropsch waxy hydrocarbon base stock(s) and/or base oil(s) are of low or zero sulfur and phosphorus content. There is a movement among original equipment manufacturers and oil formulators to produce formulated oils of ever increasingly reduced sulfated ash, phosphorus and sulfur content to meet ever increasingly restrictive environmental regulations. Such oils, known as low SAPS oils, would rely on the use of base oils which themselves, inherently, are of low or zero initial sulfur and phosphorus content. Such oils when used as base oils can be formulated with additives. Even if the additive or additives included in the formulation contain sulfur and/or phosphorus the resulting formulated lubricating oils will be lower or low SAPS oils as compared to lubricating oils formulated using conventional mineral oil base stock(s) and/or base oil(s).

For example, low SAPS formulated oils for vehicle engines (both spark ignited and compression ignited) will have a sulfur content of 0.7 wt % or less, preferably 0.6 wt % or less, more preferably 0.5 wt % or less, most preferably 0.4 wt % or less, an ash content of 1.2 wt % or less, preferably 0.8 wt % or less, more preferably 0.4 wt % or less, and a phosphorus content of 0.18% or less, preferably 0.1 wt % or less, more preferably 0.09 wt % or less, most preferably 0.08 wt % or less, and in certain instances, even preferably 0.05 wt % or less.

The base antifoaming agent(s)/defoamant(s) used in the present solution is/are one or more of any antifoaming agents/defoamants known or used by the industry to solve/treat foam problems in lubricating oil formulation compositions. Such materials typically have kinematic viscosities at 25° C. in the range of about 350 to 120,000 mm<sup>2</sup>/s or higher. "Antifoamant" may be used to designate a component that inhibits foam formation. "Defoamant" may be used to designate a component that collapses foam which has already been formed. In, practice, these terms are used interchangeably in the industry. Antifoaming agents are well-known in the art as silicone or fluorosilicone compositions, as well as certain acrylate, polyacrylate, and polymethacrylate (PMA) polymers. Such antifoaming agents useful in this invention include but are not limited to polydimethylsiloxane (PDMS) fluids and silicone polymers such as Dow Corning DCF 200 (respective viscosities at 25° C. of 60,000 mm<sup>2</sup>/s and 100,000 mm<sup>2</sup>/s), FS-1265 (1000 mm<sup>2</sup>/s), Union carbide UC-L45, polyacrylate esters such as Solutia PC-1244 and Lubrizol Lz

889D. The amount of defoaming agent in the diluent ranges from about 0.05 to 50 wt %, preferably about 0.1 wt % to about 30 wt % of the total weight of defoamant-diluent composition. The solution must be clear and bright. The stability of the defoamant-diluent composition is assessed visually (clear and bright and the absence of "fish eyes") and its effectiveness is determined in the finished lubricant over a period of time (e.g., 3 months) using conventional test methods such as the ASTM D892 and the Gearbox foam/air release test.

It has unexpectedly been discovered that GTL fluid and/or hydrodewaxed and/or hydroisomerized/catalytic (and/or solvent) dewaxed waxy feed fluid boiling between about 300 to 750° F. (149 to 399° C.), preferably between about 320 to 734° F. (160 to 390° C.), most preferably between about 320 to 700° F. (160 to 371° C.) are effective diluent fluids for the formation of stable antifoam agent/defoamant-diluent solutions.

This is unexpected because PAO base oils having boiling points within the same range and exhibiting the substantially same compositional analysis (i.e., 99-100% saturates, 0% sulfur) failed as diluents, producing solutions which were hazy and exhibited fish eye. Based on these results it would have been expected for the GTL fluid to similarly be unsuitable/unsatisfactory as a diluent oil for antifoam agents/defoamants.

The GTL fluid and/or hydrodewaxed and/or hydroisomerized/catalytic (and/or solvent) dewaxed waxy feed fluid suitable for use in the present invention are non-conventional fluids as described in detail above, boiling in the range from 300 to 750° F. (149 to 399° C.).

The antifoam agent/defoamant-GTL fluid and/or hydrodewaxed and/or hydroisomerized/catalytic (and/or solvent) dewaxed waxy feed fluid diluent solution can be added to any lubricating oil formulation composition. Such lubricating oil formulation composition can comprise the base oil as such plus antifoam agent/defoamant-diluent solution or may further contain one or more additional performance enhancing addition.

Examples of typical additives include, but are not limited to, oxidation inhibitors, antioxidants, dispersants, detergents, corrosion inhibitors, rust inhibitors, metal deactivators, anti-wear agents, extreme pressure additives, anti-seizure agents, pour point depressants, wax modifiers, viscosity index improvers, viscosity modifiers, fluid-loss additives, seal compatibility agents, friction modifiers, lubricity agents, anti-staining agents, chromophoric agents, demulsifiers, emulsifiers, densifiers, wetting agents, gelling agents, tackiness agents, colorants, and others. For a review of many commonly used additives, see Klamann in "Lubricants and Related Products", Verlag Chemie, Deerfield Beach, Fla.; ISBN 0-89573-177-0. Reference is also made to "Lubricant Additives" by M. W. Ranney, published by Noyes Data Corporation of Parkridge, N.J. (1973).

Finished lubricants comprise the lubricant base stock or base oil, plus at least one performance additive.

The types and quantities of performance additives used in combination with the instant invention in lubricant compositions are not limited by the examples shown herein as illustrations.

#### Antiwear and EP Additives

Many lubricating oils require the presence of antiwear and/or extreme pressure (EP) additives in order to provide adequate antiwear protection. Increasingly specifications for lubricant performance, e.g., engine oil performance have exhibited a trend for improved antiwear properties of the oil.

Antiwear and extreme EP additives perform this role by reducing friction and wear of metal parts.

While there are many different types of antiwear additives, for several decades the principal antiwear additive for internal combustion engine crankcase oils is a metal alkylthiophosphate and more particularly a metal dialkyldithiophosphate in which the primary metal constituent is zinc, or zinc dialkyldithiophosphate (ZDDP). ZDDP compounds generally are of the formula  $Zn[SP(S)(OR)(OR^2)]_2$  where  $R^1$  and  $R^2$  are  $C_1$ - $C_{18}$  alkyl groups, preferably  $C_2$ - $C_{12}$  alkyl groups. These alkyl groups may be straight chain or branched. The ZDDP is typically used in amounts of from about 0.4 to 1.4 wt % of the total lube oil composition, although more or less can often be used advantageously.

However, it is found that the phosphorus from these additives has a deleterious effect on the catalyst in catalytic converters and also on oxygen sensors in automobiles. One way to minimize this effect is to replace some or all of the ZDDP with phosphorus-free antiwear additives.

A variety of non-phosphorous additives are also used as antiwear additives. Sulfurized olefins are useful as antiwear and EP additives. Sulfurcontaining olefins can be prepared by sulfurization of various organic materials including aliphatic, arylaliphatic or alicyclic olefinic hydrocarbons containing from about 3 to 30 carbon atoms, preferably 3-20 carbon atoms. The olefinic compounds contain at least one non-aromatic double bond. Such compounds are defined by the formula



where each of  $R^3$ - $R^6$  are independently hydrogen or a hydrocarbon radical. Preferred hydrocarbon radicals are alkyl or alkenyl radicals. Any two of  $R^3$ - $R^6$  may be connected so as to form a cyclic ring. Additional information concerning sulfurized olefins and their preparation can be found in U.S. Pat. No. 4,941,984, incorporated by reference herein in its entirety.

The use of polysulfides of thiophosphorus acids and thiophosphorus acid esters as lubricant additives is disclosed in U.S. Pat. Nos. 2,443,264; 2,471,115; 2,526,497; and 2,591,577. Addition of phosphorothionyl disulfides as an antiwear, antioxidant, and EP additive is disclosed in U.S. Patent 3,770,854. Use of alkylthiocarbamoyl compounds in combination with a molybdenum compound (oxymolybdenum diisopropylphosphorodithioate sulfide, for example) and a phosphorous ester (dibutyl hydrogen phosphite, for example) as antiwear additives in lubricants is disclosed in U.S. Pat. No. 4,501,678. U.S. Pat. No. 4,758,362 discloses use of a carbamate additive to provide improved antiwear and extreme pressure properties. The use of thiocarbamate as an antiwear additive is disclosed in U.S. Pat. No. 5,693,598. Thiocarbamate/molybdenum complexes such as moly-sulfur alkyl dithiocarbamate trimer complex ( $R=C_8$ - $C_{18}$  alkyl) are also useful antiwear agents. The use or addition of such materials should be kept to a minimum if the object is to produce low SAPS formulations.

Esters of glycerol may be used as antiwear agents. For example, mono-, di-, and tri-oleates, mono-palmitates and mono-myristates may be used.

ZDDP is combined with other compositions that provide antiwear properties. U.S. Pat. No. 5,034,141 discloses that a combination of a thiodixanthogen compound (octylthiodixanthogen, for example) and a metal thiophosphate (ZDDP, for example) can improve antiwear properties. U.S. Pat. No. 5,034,142 discloses that use of a metal alkoxyalkylxanthate (nickel ethoxyethylxanthate, for example) and a dixanthogen

(diethoxyethyl dixanthogen, for example) in combination with ZDDP improves antiwear properties.

Preferred antiwear additives include phosphorus and sulfur compounds, such as zinc dithiophosphates and/or sulfur, nitrogen, boron, molybdenum phosphorodithioates, molybdenum dithiocarbamates and various organomolybdenum derivatives including heterocyclics, for example dimercaptothiadiazoles, mercaptobenzothiadiazoles, triazines, and the like, alicyclics, amines, alcohols, esters, diols, triols, fatty amides and the like can also be used. Such additives may be used in an amount of about 0.01 to 6 wt %, preferably about 0.01 to 4 wt %. ZDDP-like compounds provide limited hydroperoxide decomposition capability, significantly below that exhibited by compounds disclosed and claimed in this patent and can therefore be eliminated from the formulation or, if retained, kept at a minimal concentration to facilitate production of low SAPS formulations.

#### Viscosity Index Improvers

Viscosity index improvers (also known as VI improvers, viscosity modifiers, and viscosity improvers) provide lubricants with high and low temperature operability. These additives impart shear stability at elevated temperatures and acceptable viscosity at low temperatures.

Suitable viscosity index improvers include high molecular weight hydrocarbons, polyesters and viscosity index improver dispersants that function as both a viscosity index improver and a dispersant. Typical molecular weights of these polymers are between about 10,000 to 1,000,000, more typically about 20,000 to 500,000, and even more typically between about 50,000 and 200,000.

Examples of suitable viscosity index improvers are polymers and copolymers of methacrylate, butadiene, olefins, or alkylated styrenes. Polyisobutylene is a commonly used viscosity index improver. Another suitable viscosity index improver is polymethacrylate (copolymers of various chain length alkyl methacrylates, for example), some which can also serve as pour point depressants in some formulations. Other suitable viscosity index improvers include copolymers of ethylene and propylene, hydrogenated block copolymers of styrene and isoprene, and polyacrylates (copolymers of various chain length acrylates, for example). Specific examples include styrene-isoprene or styrene-butadiene based polymers of 50,000 to 200,000 molecular weight.

Viscosity index improvers may be used in an amount of about 0.01 to 8 wt %, preferably about 0.01 to 4 wt %.

#### Antioxidants

Antioxidants retard the oxidative degradation of base oils during service. Such degradation may result in deposits on metal surfaces, the presence of sludge, or a viscosity increase in the lubricant. One skilled in the art knows a wide variety of oxidation inhibitors that are useful in lubricating oil compositions. See, Klamann in "Lubricants and Related Products", op. cit., and U.S. Pat. Nos. 4,798,684 and 5,084,197, for example.

Useful antioxidants include hindered phenols. These phenolic anti-oxidants may be ashless (metal-free) phenolic compounds or neutral or basic metal salts of certain phenolic compounds. Typical phenolic antioxidant compounds are the hindered phenols which are the ones which contain a sterically-hindered hydroxyl group, and these include those derivatives of dihydroxy aryl compounds in which the hydroxyl groups are in the ortho- or para-position relative to each other. Typical phenolic antioxidants include the hindered phenols substituted with  $C_4$ -alkyl groups and the alkylene coupled derivatives of these hindered phenols. Examples of phenolic materials of this type 2-t-butyl-4-hep-

tylphenol; 2-t-butyl-4-octylphenol; 2-t-butyl-4-dodecylphenol; 2,6-di-t-butyl-4-heptylphenol; 2,6-di-t-butyl-4-dodecylphenol; 2-methyl-6-t-butyl-4-heptylphenol; and 2-methyl-6-t-butyl-4-dodecylphenol. Other useful hindered mono-phenolic antioxidants may include for example the hindered 2,6-di-alkylphenolic propionic ester derivatives. Bis-phenolic antioxidants may also be advantageously used in combination with the instant invention. Examples of ortho-coupled bisphenols include: 2,2'-bis(4-heptyl-6-t-butylphenol); 2,2'-bis(4-octyl-6-t-butylphenol); and 2,2'-bis(4-dodecyl-6-t-butylphenol). Para-coupled bisphenols include for example 4,4'-bis(2,6-di-t-butylphenol) and 4,4'-methylene-bis(2,6-di-t-butylphenol).

Non-phenolic oxidation inhibitors which may be used include aromatic amine antioxidants and these may be used either as such or in combination with phenolic antioxidants. Typical examples of non-phenolic antioxidants include: alkylated and non-alkylated aromatic amines such as aromatic monoamines of the formula  $R^8R^9R^{10}N$  where  $R^8$  is an aliphatic, aromatic or substituted aromatic group,  $R^9$  is an aromatic or a substituted aromatic group, and  $R^{10}$  is H, alkyl, aryl or  $R^{11}S(O)_xR^{12}$  where  $R^{11}$  is an alkylene, alkenylene, or aralkylene group,  $R^{12}$  is a higher alkyl group, or an alkenyl, aryl, or alkaryl group, and x is 0, 1 or 2. The aliphatic group  $R^8$  may contain from 1 to about 20 carbon atoms, and preferably contains from about 6 to 12 carbon atoms. The aliphatic group is a saturated aliphatic group. Preferably, both  $R^8$  and  $R^9$  are aromatic or substituted aromatic groups, and the aromatic group may be a fused ring aromatic group such as naphthyl. Aromatic groups  $R^8$  and  $R^9$  may be joined together with other groups such as S.

Typical aromatic amines antioxidants have alkyl substituent groups of at least about 6 carbon atoms. Examples of aliphatic groups include hexyl, heptyl, octyl, nonyl, and decyl. Generally, the aliphatic groups will not contain more than about 14 carbon atoms. The general types of amine antioxidants useful in the present compositions include diphenylamines, phenyl naphthylamines, phenothiazines, imidobenzyls and diphenyl phenylene diamines. Mixtures of two or more aromatic amines are also useful. Polymeric amine antioxidants can also be used. Particular examples of aromatic amine antioxidants useful in the present invention include: p,p'-dioctyldiphenylamine; t-octylphenyl-alpha-naphthylamine; phenyl-alpha-naphthylamine; and p-octylphenyl-alpha-naphthylamine.

Sulfurized alkyl phenols and alkali or alkaline earth metal salts thereof also are useful antioxidants.

Another class of antioxidant used in lubricating oil compositions is oil-soluble copper compounds. Any oil-soluble suitable copper compound may be blended into the lubricating oil. Examples of suitable copper antioxidants include copper dihydrocarbyl thio- or dithio-phosphates and copper salts of naturally occurring or synthetic carboxylic acids. Other suitable copper salts include copper dithiacarbamates, sulphonates, phenates, and acetylacetones. Basic, neutral, or acidic copper Cu(I) and or Cu(II) salts derived from alkenyl succinic acids or anhydrides are known to be particularly useful.

Preferred antioxidants include hindered phenols, arylamines. These antioxidants may be used individually by type or in combination with one another. Such additives may be used in an amount of about 0.01 to 5 wt %, preferably about 0.01 to 1.5 wt %.

#### Detergents

Detergents are commonly used in lubricating compositions. A typical detergent is an anionic material that contains

a long chain hydrophobic portion of the molecule and a smaller oleophobic anionic or hydrophilic portion of the molecule. The anionic portion of the detergent is typically derived from an organic acid such as a sulfur acid, carboxylic acid, phosphorus acid, phenol, or mixtures thereof. The counterion is typically an alkaline earth or alkali metal.

Salts that contain a substantially stoichiometric amount of the metal are described as neutral salts and have a total base number (TBN, as measured by ASTM D2896) of from 0 to 10 about 80. Many compositions are overbased, containing large amounts of a metal base that is achieved by reacting an excess of a metal compound (a metal hydroxide or oxide, for example) with an acidic gas (such as carbon dioxide). Useful detergents can be neutral, mildly overbased, or highly overbased.

It is desirable for at least some detergent to be overbased. Overbased detergents help neutralize acidic impurities produced by the combustion process and become entrapped in the oil. Typically, the overbased material has a ratio of metallic ion to anionic portion of the detergent of about 1.05:1 to 20 50:1 on an equivalent basis. More preferably, the ratio is from about 4:1 to about 25:1. The resulting detergent is an overbased detergent that will typically have a TBN of about 150 or higher, often about 250 to 450 or more. Preferably, the overbasing cation is sodium, calcium, or magnesium. A mixture of detergents of differing TBN can be used in the present invention.

Preferred detergents include the alkali or alkaline earth metal salts of sulfonates, phenates, carboxylates, phosphates, and salicylates.

Sulfonates may be prepared from sulfonic acids that are typically obtained by sulfonation of alkyl-substituted aromatic hydrocarbons. Hydrocarbon examples include those obtained by alkylating benzene, toluene, xylene, naphthalene, biphenyl and their halogenated derivatives (chlorobenzene, chlorotoluene, and chloronaphthalene, for example). The alkylating agents typically have about 3 to 70 carbon atoms. The alkaryl sulfonates typically contain about 9 to 35 about 80 or more carbon atoms, more typically from about 16 to 60 carbon atoms.

Klamann in "Lubricants and Related Products", op cit discloses a number of overbased metal salts of various sulfonic acids which are useful as detergents and dispersants in lubricants. The book entitled "Lubricant Additives", C. V. 45 Smallheer and R. K. Smith, published by the Lezius-Hiles Co. of Cleveland, Ohio (1967), similarly discloses a number of overbased sulfonates that are useful as dispersants and/or detergents.

Alkaline earth phenates are another useful class of detergent for lubricants. These detergents can be made by reacting alkaline earth metal hydroxide or oxide (CaO, Ca(OH)<sub>2</sub>, BaO, Ba(OH)<sub>2</sub>, MgO, Mg(OH)<sub>2</sub>, for example) with an alkyl phenol or sulfurized alkylphenol. Useful alkyl groups include straight chain or branched C<sub>1</sub>-C<sub>30</sub> alkyl groups, preferably, 55 C<sub>4</sub>-C<sub>20</sub>. Examples of suitable phenols include isobutylphenol, 2-ethylhexylphenol, nonylphenol, dodecyl phenol, and the like. It should be noted that starting alkylphenols may contain more than one alkyl substituent that are each independently straight chain or branched. When a non-sulfurized alkylphenol is used, the sulfurized product may be obtained by methods well known in the art. These methods include heating a mixture of alkylphenol and sulfurizing agent (including elemental sulfur or sulfur halides, such as sulfur dichloride, and the like) and then reacting the sulfurized phenol with an alkaline earth metal hydroxide or oxide.

Metal salts of carboxylic acids are also useful as detergents. These carboxylic acid detergents may be prepared by

reacting a basic metal compound with at least one carboxylic acid and removing free water from the reaction product. These compounds may be overbased to produce the desired TBN level. Detergents made from salicylic acid are one preferred class of detergents derived from carboxylic acids. Useful salicylates include long chain alkyl salicylates. One useful family of compositions is of the formula



where R is a hydrogen atom or an alkyl group having 1 to about 30 carbon atoms, n is an integer from 1 to 4, and M is an alkaline earth metal. Preferred R groups are alkyl chains of at least  $C_{11}$ , preferably  $C_{13}$  or greater. R may be optionally substituted with substituents that do not interfere with the detergent's function. M is preferably calcium, magnesium, or barium. More preferably, M is calcium.

Hydrocarbyl-substituted salicylic acids may be prepared from phenols by the Kolbe reaction. See U.S. Pat. No. 3,595,791, which is incorporated herein by reference in its entirety, for additional information on synthesis of these compounds. The metal salts of the hydrocarbyl-substituted salicylic acids may be prepared by double decomposition of a metal salt in a polar solvent such as water or alcohol.

Alkaline earth metal phosphates are also used as detergents.

Detergents may be simple detergents or what is known as hybrid or complex detergents. The latter detergents can provide the properties of two detergents without the need to blend separate materials. See U.S. Pat. No. 6,034,039 for example.

Preferred detergents include calcium phenates, calcium sulfonates, calcium salicylates, magnesium phenates, magnesium sulfonates, magnesium salicylates and other related components (including borated detergents). Typically, the total detergent concentration is about 0.01 to about 6.0 wt %, preferably, about 0.1 to 0.4 wt %.

#### Dispersant

During engine operation, oil-insoluble oxidation byproducts are produced. Dispersants help keep these byproducts in solution, thus diminishing their deposition on metal surfaces. Dispersants may be ashless or ash-forming in nature. Preferably, the dispersant is ashless. So-called ashless dispersants are organic materials that form substantially no ash upon combustion. For example, non-metal-containing or borated metal-free dispersants are considered ashless. In contrast, metal-containing detergents discussed above form ash upon combustion.

Suitable dispersants typically contain a polar group attached to a relatively high molecular weight hydrocarbon chain. The polar group typically contains at least one element of nitrogen, oxygen, or phosphorus. Typical hydrocarbon chains contain 50 to 400 carbon atoms.

Chemically, many dispersants may be characterized as phenates, sulfonates, sulfurized phenates, salicylates, naphthenates, stearates, carbamates, thiocarbamates, phosphorus derivatives. A particularly useful class of dispersants are the alkenylsuccinic derivatives, typically produced by the reac-

tion of a long chain substituted alkenyl succinic compound, usually a substituted succinic anhydride, with a polyhydroxy or polyamino compound. The long chain group constituting the oleophilic portion of the molecule which confers solubility in the oil, is normally a polyisobutylene group. Many examples of this type of dispersant are well known commercially and in the literature. Exemplary patents describing such dispersants are U.S. Pat. Nos. 3,172,892; 3,2145,707; 3,219,666; 3,316,177; 3,341,542; 3,444,170; 3,454,607; 3,541,012; 10 3,630,904; 3,632,511; 3,787,374 and 4,234,435. Other types of dispersant are described in U.S. Pat. Nos. 3,036,003; 3,200,107; 3,254,025; 3,275,554; 3,438,757; 3,454,555; 3,565,804; 3,413,347; 3,697,574; 3,725,277; 3,725,480; 3,726,882; 4,454,059; 3,329,658; 3,449,250; 3,519,565; 3,666,730; 15 3,687,849; 3,702,300; 4,100,082; 5,705,458. A further description of dispersants may be found, for example, in European Patent Application No. 471 071, to which reference is made for this purpose.

Hydrocarbyl-substituted succinic acid compounds are 20 popular dispersants. In particular, succinimide, succinate esters, or succinate ester amides prepared by the reaction of a hydrocarbon-substituted succinic acid compound preferably having at least 50 carbon atoms in the hydrocarbon substituent, with at least one equivalent of an alkylene amine are 25 particularly useful.

Succinimides are formed by the condensation reaction between alkenyl succinic anhydrides and amines. Molar ratios can vary depending on the polyamine. For example, the molar ratio of alkenyl succinic anhydride to TEPA can vary 30 from about 1:1 to about 5:1. Representative examples are shown in U.S. Pat. Nos. 3,087,936; 3,172,892; 3,219,666; 3,272,746; 3,322,670; and 3,652,616, 3,948,800; and Canada Patent No. 1,094,044.

Succinate esters are formed by the condensation reaction 35 between alkenyl succinic anhydrides and alcohols or polyols. Molar ratios can vary depending on the alcohol or polyol used. For example, the condensation product of an alkenyl succinic anhydride and pentaerythritol is a useful dispersant.

Succinate ester amides are formed by condensation reaction 40 between alkenyl succinic anhydrides and alkanol amines. For example, suitable alkanol amines include ethoxylated polyalkylpolyamines, propoxylated polyalkylpolyamines and polyalkenylpolyamines such as polyethylene polyamines. One example is propoxylated hexamethylenediamine. Representative examples are shown in U.S. Pat. No. 4,426,305.

The molecular weight of the alkenyl succinic anhydrides used in the preceding paragraphs will typically range between 50 800 and 2,500. The above products can be post-reacted with various reagents such as sulfur, oxygen, formaldehyde, carboxylic acids such as oleic acid, and boron compounds such as borate esters or highly borated dispersants. The dispersants can be borated with from about 0.1 to about 5 moles of boron per mole of dispersant reaction product.

Mannich base dispersants are made from the reaction of 55 alkenylphenols, formaldehyde, and amines. See U.S. Pat. No. 4,767,551, which is incorporated herein by reference. Process aids and catalysts, such as oleic acid and sulfonic acids, can also be part of the reaction mixture. Molecular weights of the alkenylphenols range from 800 to 2,500. Representative examples are shown in U.S. Pat. Nos. 3,697,574; 3,703,536; 3,704,308; 3,751,365; 3,756,953; 3,798,165; and 3,803,039.

Typical high molecular weight aliphatic acid modified 60 Mannich condensation products useful in this invention can be prepared from high molecular weight alkyl-substituted hydroxyaromatics or  $HN(R)_2$  group-containing reactants.

Examples of high molecular weight alkyl-substituted hydroxyaromatic compounds are polypropylphenol, polybutylphenol, and other polyalkylphenols. These polyalkylphenols can be obtained by the alkylation, in the presence of an alkylating catalyst, such as  $\text{BF}_3$ , of phenol with high molecular weight poly-propylene, polybutylene, and other polyalkylene compounds to give alkyl substituents on the benzene ring of phenol having an average 600-100,000 molecular weight.

Examples of  $\text{HN}(\text{R})_2$  group-containing reactants are alkylene polyamines, principally polyethylene polyamines. Other representative organic compounds containing at least one  $\text{HN}(\text{R})_2$  group suitable for use in the preparation of Mannich condensation products are well known and include the mono- and di-aminoalkanes and their substituted analogs, e.g., ethylamine and diethanolamine; aromatic diamines, e.g., phenylenediamine, diamino naphthalenes; heterocyclic amines, e.g., morpholine, pyrrole, pyrrolidine, imidazole, imidazoline, and piperidine; melamine and their substituted analogs.

Examples of alkylene polyamide reactants include ethylenediamine, diethylene triamine, triethylene tetraamine, tetraethylene pentaamine, pentaethylene hexamine, hexaethylene heptaamine, heptaethylene octaamine, octaethylene nonaamine, nonaethylene decamine, and decaethylene undecamine and mixture of such amines having nitrogen contents corresponding to the alkylene polyamines, in the formula  $\text{H}_2\text{N}-(\text{Z}-\text{NH})_n\text{H}$ , mentioned before, Z is a divalent ethylene and n is 1 to 10 of the foregoing formula. Corresponding propylene polyamines such as propylene diamine and di-, tri-, tetra-, pentapropylene tri-, tetra-, penta- and hexaamines are also suitable reactants. The alkylene polyamines are usually obtained by the reaction of ammonia and dihalo alkanes, such as dichloro alkanes. Thus the alkylene polyamines obtained from the reaction of 2 to 11 moles of ammonia with 1 to 10 moles of dichloroalkanes having 2 to 6 carbon atoms and the chlorines on different carbons are suitable alkylene polyamine reactants.

Aldehyde reactants useful in the preparation of the high molecular products useful in this invention include the aliphatic aldehydes such as formaldehyde (also known as paraformaldehyde and formalin), acetaldehyde and aldol ( $\beta$ -hydroxybutyraldehyde). Formaldehyde or a formaldehyde-yielding reactant is preferred.

Hydrocarbyl substituted amine ashless dispersant additives are well known to one skilled in the art; see, for example, U.S. Pat. Nos. 3,275,554; 3,438,757; 3,565,804; 3,755,433, 3,822,209, and 5,084,197.

Preferred dispersants include borated and non-borated succinimides, including those derivatives from mono-succinimides, bis-succinimides, and/or mixtures of mono- and bis-succinimides, wherein the hydrocarbyl succinimide is derived from a hydrocarbylene group such as polyisobutylene having a Mn from about 500 to about 5000 or a mixture of such hydrocarbylene groups. Other preferred dispersants include succinic acid-esters and amides, alkylphenolpolyamine-coupled Mannich adducts, their capped derivatives, and other related components. Such additives may be used in an amount of about 0.1 to 20 wt %, preferably about 0.1 to 8 wt %.

#### Pour Point Depressants

Conventional pour point depressants (also known as lube oil flow improvers) may be added to the compositions of the present invention if desired. These pour point depressants may be added to lubricating compositions of the present invention to lower the minimum temperature at which the fluid will flow or can be poured. Examples of suitable pour point depressants include alkylated naphthalene, poly-

methacrylates, polyacrylates, polyarylamides, condensation products of haloparaffin waxes and aromatic compounds, vinyl carboxylate polymers, and terpolymers of dialkylfumarates, vinyl esters of fatty acids and allyl vinyl ethers. U.S.

5 Pat. Nos. 1,815,022; 2,015,748; 2,191,498; 2,387,501; 2,655, 479; 2,666,746; 2,721,877; 2,721,878; and 3,250,715 describe useful pour point depressants and/or the preparation thereof. Such additives may be used in an amount of about 0.01 to 5 wt %, preferably about 0.01 to 1.5 wt %.

#### 10 Corrosion Inhibitors

Corrosion inhibitors are used to reduce the degradation of metallic parts that are in contact with the lubricating oil composition. Suitable corrosion inhibitors include thiadiazoles. See, for example, U.S. Pat. Nos. 2,719,125; 2,719,126; and 3,087,932. Such additives may be used in an amount of about 0.01 to 5 wt %, preferably about 0.01 to 1.5 wt %.

#### Seal Compatibility Additives

Seal compatibility agents help to swell elastomeric seals by 20 causing a chemical reaction in the fluid or physical change in the elastomer. Suitable seal compatibility agents for lubricating oils include organic phosphates, aromatic esters, aromatic hydrocarbons, esters (butylbenzyl phthalate, for example), and polybutenyl succinic anhydride. Such additives may be used in an amount of about 0.01 to 3 wt %, preferably about 0.01 to 2 wt %.

#### Inhibitors and Antirust Additives

30 Antirust additives (or corrosion inhibitors) are additives that protect lubricated metal surfaces against chemical attack by water or other contaminants. A wide variety of these are commercially available; they are referred to in Klamann in "Lubricants and Related Products", op cit.

One type of antirust additive is a polar compound that wets the metal surface preferentially, protecting it with a film of oil. Another type of antirust additive absorbs water by incorporating it in a water-in-oil emulsion so that only the oil touches the metal surface. Yet another type of antirust additive chemically adheres to the metal to produce a non-reactive surface. Examples of suitable additives include zinc dithiophosphates, metal phenolates, basic metal sulfonates, fatty acids and amines. Such additives may be used in an amount of about 0.01 to 5 wt %, preferably about 0.01 to 1.5 wt %.

#### Friction Modifiers

45 A friction modifier is any material or materials that can alter the coefficient of friction of a surface lubricated by any lubricant or fluid containing such material(s). Friction modifiers, also known as friction reducers, lubricity agents or oiliness agents, and other such agents that change the ability of base oils, formulated lubricant compositions, or functional fluids, to modify the coefficient of friction of a lubricated surface may be effectively used in combination with the base oils or lubricant compositions of the present invention if desired. Friction modifiers that lower the coefficient of friction 50 are particularly advantageous in combination with the base oils and lube compositions of this invention. Friction modifiers may include metal-containing compounds or materials as well as ashless compounds or materials, or mixtures thereof. Metal-containing friction modifiers may include

55 metal salts or metalligand complexes where the metals may include alkali, alkaline earth, or transition group metals. Such metal-containing friction modifiers may also have low-ash characteristics. Transition metals may include Mo, Sb, Sn, Fe, Cu, Zn, and others. Ligands may include hydrocarbyl derivative of alcohols, polyols, glycerols, partially esterified glycerols, thiols, carboxylates, carbamates, thiocarbamates, dithiocarbamates, phosphates, thiophosphates, dithiophos-

phates, amides, imides, amines, thiazoles, thiadiazoles, dithiazoles, diazoles, triazoles, and other polar molecular functional groups containing effective amounts of O, N, S, or P, individually or in combination. In particular, Mo-containing compounds can be particularly effective as for example Mo-dithiocarbamates, Mo(DTC), Mo-dithiophosphates, Mo(DTP), Mo-amines, Mo (Am), Mo-alcoholates, Mo-alcohol-amides, etc. See U.S. Pat. Nos. 5,824,627; 6,232,276; 6,153,564; 6,143,701; 6,110,878; 5,837,657; 6,010,987; 5,906,968; 6,734,150; 6,730,638; 6,689,725; 6,569,820; and WO 99/66013; WO 99/47629; WO 98/26030.

Ashless friction modifiers may also include lubricant materials that contain effective amounts of polar groups, for example, hydroxyl-containing hydrocarbyl base oils, glycerides, partial glycerides, glyceride derivatives, and the like. Polar groups in friction modifiers may include hydrocarbyl groups containing effective amounts of O, N, S, or P, individually or in combination. Other friction modifiers that may be particularly effective include, for example, salts (both ash-containing and ashless derivatives) of fatty acids, fatty alcohols, fatty amides, fatty esters, hydroxyl-containing fatty carboxylates, and comparable synthetic long-chain hydrocarbyl acids, alcohols, amides, esters, hydroxy carboxylates, and the like. In some instances fatty organic acids, fatty amines, and sulfurized fatty acids may be used as suitable friction modifiers.

Useful concentrations of friction modifiers may range from about 0.01 to 10-15 wt % or more, often with a preferred range of about 0.1 to 5 wt %. Concentrations of molybdenum-containing friction modifiers are often described in terms of Mo metal concentration. Advantageous concentrations of Mo may range from about 10 to 3000 ppm or more, and often with a preferred range of about 20 to 2000 ppm, and in some instances a more preferred range of about 30 to 1000 ppm. Friction modifiers of all types may be used alone or in mixtures with the materials of this invention. Often mixtures of two or more friction modifiers, or mixtures of friction modifier(s) with alternate surface active material(s), are also desirable.

#### Typical Additive Amounts

When lubricating oil compositions contain one or more of the additives discussed above, the additive(s) are blended into the composition in an amount sufficient for it to perform its intended function. Typical amounts of such additives useful in the present invention are shown in Table 1 below.

Note that many of the additives are shipped from the manufacturer and used with a certain amount of diluent base oil solvent in the formulation. Accordingly, the weight amounts in the table below, as well as other amounts mentioned in this text, are directed to the amount of active ingredient (that is the non-diluent/solvent portion of the ingredient) unless otherwise indicated. The weight percent indicated below are based on the total weight of the lubricating oil composition.

TABLE 1

| Typical Amounts of Various Lubricant Oil Components |                           |                                  |
|-----------------------------------------------------|---------------------------|----------------------------------|
| Compound                                            | Approximate Wt % (Useful) | Approximate Wt % (Preferred)     |
| Detergent                                           | 0.01-6                    | 0.01-4                           |
| Dispersant                                          | 0.1-20                    | 0.1-8                            |
| Friction Reducer                                    | 0.01-5                    | 0.01-1.5                         |
| Viscosity                                           | 0.0-40                    | 0.01-30, more preferably 0.01-15 |
| Index Improver                                      | 0.0-5                     | 0.01-15                          |
| Antioxidant                                         | 0.0-5                     | 0.0-1.5                          |
| Corrosion Inhibitor                                 | 0.01-5                    | 0.01-1.5                         |

TABLE 1-continued

| Typical Amounts of Various Lubricant Oil Components |                           |                              |
|-----------------------------------------------------|---------------------------|------------------------------|
| Compound                                            | Approximate Wt % (Useful) | Approximate Wt % (Preferred) |
| Anti-wear Additive                                  | 0.01-6                    | 0.01-4                       |
| Pour Point Depressant                               | 0.0-5                     | 0.01-1.5                     |
| Base Oil                                            | Balance                   | Balance                      |

10

The present invention is further defined and demonstrated by the following non-limiting examples and comparisons.

#### EXAMPLE 1

Method: 1.2 vol % of 60,000 cSt polydimethylsiloxane (DCF 200) was dissolved in 98.8 vol % of the test diluent. The stability of the defoamer-diluent mixture was assessed visually for clarity and brightness (clear and bright) and absence of "fish eyes" over a period of 3 weeks. The results show that the Fail/Pass criteria cannot be predicted based on the diluent composition. The PAOs are 100% saturates and when used as diluent produced a solution which did not meet the Clear and Bright criteria despite coming closest to matching the GTL oil in terms of saturates and sulfur content.

TABLE 2

| Diluent                                                    | Composition                                                                                                            | Visual Observation after 3 weeks |
|------------------------------------------------------------|------------------------------------------------------------------------------------------------------------------------|----------------------------------|
| Pluronic L81                                               | Polyglycol                                                                                                             | F                                |
| Aromatic 100                                               | 99.6% Aromatics, 0.4% Saturates                                                                                        | P                                |
| Aromatic 200                                               | 99.6% Aromatics, 0.4% Saturates                                                                                        | F                                |
| SpectraSyn 2 (PAO)                                         | 100% Saturates 0% S                                                                                                    | F                                |
| Synesstic 5                                                | Alkylated naphthalene                                                                                                  | F                                |
| Synesstic 12                                               | Alkylated naphthalene                                                                                                  | F                                |
| Esterex A32                                                | Adipate ester                                                                                                          | F                                |
| Zerol 150                                                  | Alkylated benzenes                                                                                                     | F                                |
| Zerol 500                                                  | Alkylated benzenes                                                                                                     | F                                |
| Isopar L                                                   | 91% Paraffins, 9% Cycloparaffins                                                                                       | P                                |
| Exxsol D110                                                | 45% Cycloparaffins, 55% Paraffins <0.5% Aromatics                                                                      | P                                |
| Exxsol D60                                                 | 58% Cycloparaffins, 42% Paraffins <0.5% Aromatics                                                                      | P                                |
| Kerosene (Jet A Fuel) (High sulfur)                        | 25% Isoparaffins, 22% Paraffins, 23% Aromatics, 30% Cycloparaffins                                                     | P                                |
| Jet A (Kerosene) (Low sulfur) (GTL)(invention)             | 24% Isoparaffins, 21% Paraffins, 23% Aromatics, 32% Cycloparaffins >99% Saturates, 0% Sulfur 302-536° F. (150-280° C.) | P                                |
| KV at 40° C. about 2.6 mm <sup>2</sup> /s (GTL)(invention) | >99% Saturates, 0% Sulfur 320-698° F. (160-370° C.)                                                                    | P*                               |

55 P = Pass (Clear &amp; Bright)

F = Fail (Fish eyes or not Clear &amp; Bright).

\*After 6 months both defoamer-diluent mixtures are Clear &amp; Bright.

#### EXAMPLE 2

Following Example 1, those combinations of defoamer/diluent fluid which were found to be clear and bright and did not exhibit "fish eyes" were evaluated for their antifoam/defoamant performance in a circulating lubricating oil formulation.

If the defoamer-diluent mixture was still bright and clear with no drop out or fish eyes, the defoamer mixture was

formulated in a turbine oil formulation and the foaming properties measured by the ASTM D 892 Sequence I test method over a period of about 80 days.

| ISO 68 Mineral-Based Turbine/Circulating Oil |        |
|----------------------------------------------|--------|
| Components                                   | Wt %   |
| Base Stocks                                  | 99.035 |
| Defoamer                                     | 0.005  |
| Other Additives                              | 0.995  |

The circulating oil comprises a mixture of Group I base stock (about 20.0 wt %) and Group II base stocks (about 79.0 wt %). Beside the 0.005 wt % defoamer/diluent solution, it contained about 0.960 wt % additives.

Defoamer=1 wt % of DCF 200 in diluents shown in Table 3.

TABLE 3

| Foaming Tendency, Seq I, mL |                       |                      |                 |             |                |                       |                      |                      |
|-----------------------------|-----------------------|----------------------|-----------------|-------------|----------------|-----------------------|----------------------|----------------------|
| Days                        | High S<br>Jet A<br>98 | Low S<br>Jet A<br>04 | Aromatic<br>100 | Isopar<br>L | Exxsol<br>D110 | High<br>S Jet<br>A 04 | GTL<br>(320-698° F.) | GTL<br>(302-536° F.) |
| 0                           | 0                     | 0                    | 15              | 0           | 0              | 0                     | 0                    | 0                    |
| 16                          | —                     | —                    | —               | —           | —              | —                     | 0                    | 0                    |
| 42                          | —                     | —                    | —               | —           | —              | —                     | 0                    | 0                    |
| 45                          | 0                     | 30                   | 120             | 25          | 20             | 10                    | —                    | —                    |
| 60                          | 90                    | 95                   | 155             | 70          | 55             | 20                    | —                    | —                    |
| 75                          | 180                   | 160                  | 190             | 120         | 90             | 15                    | —                    | —                    |
| 77                          | —                     | —                    | —               | —           | —              | —                     | —                    | 0                    |
| 83                          | —                     | —                    | —               | —           | —              | 0                     | —                    | —                    |

As can be seen, not only does the GTL fluid (possessing 99% saturates and % sulfur) function as an effective diluent whereas PAO which is 100% saturate and also contains zero % sulfur failed as a diluent (haze and fish eyes exhibited when PAO was used as a diluent), but the antifoam/defoamant-GTL fluid diluent solution when tested for its ability to perform its antifoam/defoamant function in a lubricating oil formulation far exceeded the performance of other solutions which had also passed the clear and bright visual test but which were drastically different compositionally.

The ability of GTL fluid and/or hydrodewaxed and/or hydroisomerized/catalytic (and/or solvent) dewaxed waxy feed derived fluid to perform as a diluent oil to form a stable antifoam/defoamant-diluent oil solution, whereas PAO failed as a diluent solution despite also being near 100% paraffinic and possessing zero % sulfur, and for the solution to exhibit superior antifoam/defoamant performance in comparison to other soluble systems wherein the diluent oils were drastically different compositionally is indicative of the unexpected nature of the present invention.

What is claimed is:

1. A stable defoamant solution comprising a defoamant/antifoam agent dissolved in a diluent fluid wherein the diluent fluid is selected from the group consisting of GTL fluid, hydrodewaxed waxy feed fluid, hydroisomerized/catalytic (and/or solvent) dewaxed waxy feed derived fluid and mixtures thereof, wherein said fluid is characterized by boiling in the range of about 300° F. to about 750° F. the range recited corresponding to the initial boiling point (IBP) and to the final boiling point (FBP) of the diluent fluid and a kinematic viscosity (KV) at 40° C. in the range of about 1.2 to 4.5 mm<sup>2</sup>/s,

wherein the defoamant/antifoam agent is present in the defoamant solution in an amount in the range of from about 0.05 to about 50 wt % and the defoamant/antifoam agent is selected from the group consisting of silicone and fluorosilicone defoamant/antifoam agent compositions and wherein the defoamant solution is characterized as being clear and bright and marked by the absence of fish eyes over a period of three weeks.

2. The stable defoamant solution of claim 1 wherein the defoamant/antifoam agent is present in the defoamant solution in an amount of from 0.1 to about 30 wt %.

3. The stable defoamant solution of claim 2 wherein the defoamant/antifoam agent is present in the defoamant solution in an amount in the range of from about 0.1 to about 5 wt %.

4. A method for controlling the foam in lubricating oil compositions comprising one or more natural synthetic, or non-conventional base stocks and at least one performance

additive said method comprising adding to the lubricating oil formulation the defoamant solution according to claim 1 wherein the foam is held to zero ml as measured by the ASTMD 892 Sequence 1 method over a period of about 80 days.

5. The method of claim 4 wherein the defoamant solution added to the lubricating oil composition is the defoamant solution is characterized as being clear and bright after six months.

6. The method of claim 4 wherein the diluent in the defoamant solution added to the lubricating oil composition is a GTL fluid characterized by having a kinematic viscosity (KV) at 40° C. in the range of about 1.2 to 4.50 mm<sup>2</sup>/s.

7. The method of claim 4 wherein the defoamant solution added to the lubricating oil composition in an amount in the range of about 0.001 to 0.5 wt % based on the total weight of the finished lubricating oil composition.

8. The stable defoamant solution of claim 1 wherein the defoamant/antifoam agent is selected from polydimethylsiloxane and silicone polymers.

9. The stable defoamant solution of claim 1, 2, 3 or 8 wherein the GTL fluid, hydrodewaxed waxy feed fluid, hydroisomerized/catalytic (and/or solvent) dewaxed waxy feed fluid, or mixture thereof is characterized by boiling in the range of about 320° F. to about 734° F.

10. The stable defoamant solution of claim 9 wherein the diluent is a GTL fluid.

11. The stable defoamant solution of claim 10 wherein the diluent fluid is further characterized by having a kinematic viscosity (KV) at 40° C. in the range of about 1.2 to 4.50 mm<sup>2</sup>/s.

**31**

12. The stable defoamant solution of claim **11** wherein the diluent fluid is further characterized by having a kinematic viscosity (KV) at 40° C. in the range of about 1.2 to 3.0 mm<sup>2</sup>/s.

13. The stable defoamant solution of claim **1, 2, 3 or 8** wherein the defoamant solution is characterized as being clear and bright after six months.

14. The stable defoamant solution of claim **13** wherein the diluent fluid is further characterized by having a kinematic viscosity (KV) at 40° C. in the range of about 1.2 to 4.5 10 mm<sup>2</sup>/s.

5

**32**

15. The stable defoamant solution of claim **1, 2, 3, or 8** wherein the diluent fluid is further characterized by having a kinematic viscosity (KV) at 40° C. in the range of about 1.7 to 3.0 mm<sup>2</sup>/s.

16. The stable defoamant solution of claim **1, 2, 3 or 8** wherein the diluent fluid is further characterized by having a kinematic viscosity (KV) at 40° C. in the range of about 1.9 to 2.5 mm<sup>2</sup>/s.

\* \* \* \* \*